



US008821653B2

(12) **United States Patent**  
**Anelli et al.**

(10) **Patent No.:** **US 8,821,653 B2**  
(b5) **Date of Patent:** **Sep. 2, 2014**

(54) **HEAVY WALL STEEL PIPES WITH EXCELLENT TOUGHNESS AT LOW TEMPERATURE AND SULFIDE STRESS CORROSION CRACKING RESISTANCE**

3,810,793 A 5/1974 Heller  
3,915,697 A 10/1975 Giuliani et al.  
4,231,555 A 11/1980 Saito  
4,336,081 A 6/1982 Hijikata et al.

(Continued)

(75) Inventors: **Ettore Anelli**, Bergamo (IT); **Mariano Armengol**, Bergamo (IT); **Paolo Novelli**, Bergamo (IT); **Federico Tintori**, Bergamo (IT)

## FOREIGN PATENT DOCUMENTS

AR 0050159 A1 10/2006  
CN 1401809 3/2003

(Continued)

(73) Assignee: **Dalmine S.p.A.**, Bergamo (IT)

(\*) Notice: Subject to any disclaimer, the term of this patent is extended or adjusted under 35 U.S.C. 154(b) by 46 days.

(21) Appl. No.: **13/367,312**

## OTHER PUBLICATIONS

(22) Filed: **Feb. 6, 2012**

Machine-English translation of JP 2000-178645, Jun. 27, 2000, Ichinose Takeshi.\*

(65) **Prior Publication Data**

US 2012/0204994 A1 Aug. 16, 2012

(Continued)

(30) **Foreign Application Priority Data**

Feb. 7, 2011 (IT) ..... MI2011A0179

Primary Examiner — Deborah Yee

(51) **Int. Cl.**  
C22C 38/44 (2006.01)  
C22C 38/46 (2006.01)  
C21D 8/10 (2006.01)  
C21D 9/08 (2006.01)

(74) Attorney, Agent, or Firm — Knobbe Martens Olson & Bear, LLP

(52) **U.S. Cl.**  
USPC ..... 148/335; 148/593; 148/909; 138/177

## ABSTRACT

(58) **Field of Classification Search**  
USPC ..... 148/335, 593, 909; 420/108, 109, 111;  
138/177

Embodiments of the present disclosure comprise carbon steels and methods of manufacturing thick walled pipes (wall thickness greater than or equal to about 35 mm) there from. In one embodiment, a steel composition is processed that yields an average prior austenite grain size greater than about 15 or 20  $\mu\text{m}$  and smaller than about 100  $\mu\text{m}$ . Using this composition, a quenching sequence is provided that yields a microstructure of greater than or equal to about 50% by volume, and less than or equal to about 50% by volume, lower bainite, without substantial ferrite, upper bainite, or granular bainite. After quenching, pipes may be tempered. The quenched and tempered pipes may exhibit yield strengths greater than about 450 MPa (65 ksi) or 485 (70 ksi). Mechanical property measurements find the quenched and tempered pipes suitable for 450 MPa grade and 485 MPa grade, and resistance to sulfide stress corrosion cracking.

(56) **References Cited**

27 Claims, 8 Drawing Sheets

## U.S. PATENT DOCUMENTS

3,413,166 A 11/1968 Zackay et al.  
3,655,465 A 4/1972 Snape et al.



| (56)                  | References Cited |                          |                      |         |                |  |
|-----------------------|------------------|--------------------------|----------------------|---------|----------------|--|
| U.S. PATENT DOCUMENTS |                  |                          |                      |         |                |  |
| 4,376,528 A           | 3/1983           | Ohshimatai et al.        | 2010/0136363 A1      | 6/2010  | Valdez et al.  |  |
| 4,379,482 A           | 4/1983           | Suzuki et al.            | 2010/0193085 A1      | 8/2010  | Garcia         |  |
| 4,407,681 A           | 10/1983          | Ina et al.               | 2010/0294401 A1      | 11/2010 | Gomez          |  |
| 4,526,628 A           | 7/1985           | Ohno et al.              | 2010/0319814 A1      | 12/2010 | Perez          |  |
| 4,721,536 A           | 1/1988           | Koch et al.              | 2010/0327550 A1      | 12/2010 | Lopez          |  |
| 4,812,182 A           | 3/1989           | Fang et al.              | 2011/0097235 A1      | 4/2011  | Turconi et al. |  |
| 4,814,141 A           | 3/1989           | Imai et al.              | 2011/0247733 A1      | 10/2011 | Arai et al.    |  |
| 5,352,406 A           | 10/1994          | Barteri et al.           | 2013/0264123 A1      | 10/2013 | Altschuler     |  |
| 5,454,883 A           | 10/1995          | Yoshie et al.            |                      |         |                |  |
| 5,538,566 A           | 7/1996           | Gallagher                | CN 1487112           | 4/2004  |                |  |
| 5,592,988 A           | 1/1997           | Meroni et al.            | CN 101613829 A       | 12/2009 |                |  |
| 5,598,735 A           | 2/1997           | Saito et al.             | CN 101413089         | 11/2010 |                |  |
| 5,879,474 A           | 3/1999           | Bhadeshia et al.         | EP 0 092 815         | 11/1983 |                |  |
| 5,944,921 A           | 8/1999           | Cumino et al.            | EP 0 658 632         | 6/1995  |                |  |
| 5,993,570 A           | 11/1999          | Gray                     | EP 0 753 595         | 1/1997  |                |  |
| 6,030,470 A           | 2/2000           | Hensger et al.           | EP 0 828 007 A1      | 3/1998  |                |  |
| 6,188,037 B1          | 2/2001           | Hamada et al.            | EP 0 989 196         | 3/2000  |                |  |
| 6,196,530 B1          | 3/2001           | Muhr et al.              | EP 01027944 B1       | 8/2000  |                |  |
| 6,217,676 B1          | 4/2001           | Takabe et al.            | EP 1 277 848         | 1/2003  |                |  |
| 6,248,187 B1          | 6/2001           | Asahi et al.             | EP 1 288 316         | 3/2003  |                |  |
| 6,267,828 B1          | 7/2001           | Kushida et al.           | EP 1 413 639         | 4/2004  |                |  |
| 6,311,965 B1          | 11/2001          | Muhr et al.              | EP 1 717 324         | 11/2006 |                |  |
| 6,384,388 B1          | 5/2002           | Anderson et al.          | EP 1 914 324         | 4/2008  |                |  |
| 6,514,359 B2          | 2/2003           | Kawano                   | EP 2 028 284         | 2/2009  |                |  |
| 6,632,296 B2          | 10/2003          | Yoshinaga et al.         | EP 2133442 A1        | 12/2009 |                |  |
| 6,648,991 B2          | 11/2003          | Turconi et al.           | JP 60-086209         | 5/1985  |                |  |
| 6,669,285 B1          | 12/2003          | Park et al.              | JP 60-215719         | 10/1985 |                |  |
| 6,669,789 B1          | 12/2003          | Edelman et al.           | JP 36025719          | 10/1985 |                |  |
| 6,682,610 B1          | 1/2004           | Inoue                    | JP 61270355          | 11/1986 |                |  |
| 6,683,834 B2          | 1/2004           | Ohara et al.             | JP 63004046 A2       | 1/1988  |                |  |
| 6,709,534 B2          | 3/2004           | Kusinski et al.          | JP 63004047 A2       | 1/1988  |                |  |
| 6,767,417 B2          | 7/2004           | Fujita et al.            | JP 63230847 A2       | 9/1988  |                |  |
| 6,958,099 B2          | 10/2005          | Nakamura et al.          | JP 63230851 A2       | 9/1988  |                |  |
| 7,074,283 B2          | 7/2006           | Omura                    | JP 01 259124 A2      | 10/1989 |                |  |
| 7,083,686 B2          | 8/2006           | Itou                     | JP 01 259125 A2      | 10/1989 |                |  |
| 7,118,637 B2          | 10/2006          | Kusinski et al.          | JP 01 283322 A2      | 11/1989 |                |  |
| 7,214,278 B2          | 5/2007           | Kusinski et al.          | JP 05-098350         | 12/1990 |                |  |
| 7,264,684 B2          | 9/2007           | Numata et al.            | JP 403006329 A       | 1/1991  |                |  |
| 7,635,406 B2          | 12/2009          | Numata et al.            | JP 04 021718 A2      | 1/1992  |                |  |
| 7,744,708 B2          | 6/2010           | López et al.             | JP 04 107214         | 4/1992  |                |  |
| 7,862,667 B2          | 1/2011           | Turconi et al.           | JP 04 231414 A2      | 8/1992  |                |  |
| 8,002,910 B2          | 8/2011           | Tivelli et al.           | JP 05 287381 A2      | 11/1993 |                |  |
| 8,007,601 B2          | 8/2011           | López et al.             | JP 06-093339         | 4/1994  |                |  |
| 8,007,603 B2          | 8/2011           | Garcia et al.            | JP 06 172859 A2      | 6/1994  |                |  |
| 8,016,362 B2          | 9/2011           | Itoga                    | JP 06-220536         | 8/1994  |                |  |
| 8,317,946 B2 *        | 11/2012          | Arai et al. .... 148/335 | JP 07 041856 A2      | 2/1995  |                |  |
| 8,414,715 B2          | 4/2013           | Altschuler et al.        | JP 07 197125 A2      | 8/1995  |                |  |
| 2001/0035235 A1       | 11/2001          | Kawano                   | JP 08 311551         | 11/1996 |                |  |
| 2002/0011284 A1       | 1/2002           | Von Hagen et al.         | JP 09 067624 A2      | 3/1997  |                |  |
| 2003/0019549 A1       | 1/2003           | Turconi et al.           | JP 09-235617         | 9/1997  |                |  |
| 2003/0111146 A1       | 6/2003           | Kusinski et al.          | JP 10 140250         | 5/1998  |                |  |
| 2003/0116238 A1       | 6/2003           | Fujita                   | JP 10 176239         | 6/1998  |                |  |
| 2003/0155052 A1       | 8/2003           | Kondo et al.             | JP 10 280037 A       | 10/1998 |                |  |
| 2003/0165098 A1       | 9/2003           | Ohara et al.             | JP 11 050148 A       | 2/1999  |                |  |
| 2004/0118490 A1       | 6/2004           | Klueh et al.             | JP 11140580          | 5/1999  |                |  |
| 2004/0131876 A1       | 7/2004           | Ohgami et al.            | JP 11229079          | 8/1999  |                |  |
| 2004/0139780 A1       | 7/2004           | Cai et al.               | JP 2000-063940       | 2/2000  |                |  |
| 2005/0076975 A1       | 4/2005           | Lopez et al.             | JP 2000-313919 A2    | 11/2000 |                |  |
| 2005/0087269 A1       | 4/2005           | Merwin                   | JP 2001-131698       | 5/2001  |                |  |
| 2006/0124211 A1       | 6/2006           | Takano et al.            | JP 2001-164338       | 6/2001  |                |  |
| 2006/0137781 A1       | 6/2006           | Kusinski et al.          | JP 2001-172739 A2    | 6/2001  |                |  |
| 2006/0169368 A1       | 8/2006           | Lopez et al.             | JP 2001-271134       | 10/2001 |                |  |
| 2006/0243355 A1       | 11/2006          | Haiderer et al.          | JP 2002-096105 A2    | 4/2002  |                |  |
| 2007/0089813 A1       | 4/2007           | Tivelli                  | JP 2004-011009       | 1/2004  |                |  |
| 2007/0137736 A1       | 6/2007           | Omura et al.             | JP 60 174822 A       | 9/2005  |                |  |
| 2007/0216126 A1       | 9/2007           | Lopez et al.             | KR 0245031           | 3/2000  |                |  |
| 2008/0047635 A1       | 2/2008           | Konda et al.             | WO WO 96/22396       | 7/1996  |                |  |
| 2008/0129044 A1       | 6/2008           | Carcagno et al.          | WO WO 00/70107       | 11/2000 |                |  |
| 2008/0219878 A1       | 9/2008           | Konda et al.             | WO WO 01/88210       | 11/2001 |                |  |
| 2008/0226396 A1       | 9/2008           | Garcia et al.            | WO WO 03/033856      | 4/2003  |                |  |
| 2008/0226491 A1       | 9/2008           | Satou et al.             | WO WO 2004/031420    | 4/2004  |                |  |
| 2008/0314481 A1       | 12/2008          | Garcia et al.            | WO WO 2004/097059 A1 | 11/2004 |                |  |
| 2009/0010794 A1       | 1/2009           | Turconi et al.           | WO WO 2007/017161    | 2/2007  |                |  |
| 2009/0101242 A1       | 4/2009           | Lopez et al.             | WO WO 2008/003000    | 1/2008  |                |  |
| 2010/0068549 A1       | 3/2010           | Agazzi                   | WO WO 2008/127084 A2 | 10/2008 |                |  |

## FOREIGN PATENT DOCUMENTS

(56)

## References Cited

## FOREIGN PATENT DOCUMENTS

WO WO 2009/044297 4/2009  
 WO WO 2010/061882 A1 6/2010

## OTHER PUBLICATIONS

- “Seamless Steel Tubes for Pressure Purposes—Technical Delivery Conditions—Part 1: Non-alloy Steel Tubes with Specified Room Temperature Properties” British Standard BS EN 10216-1:2002 E:1-26, published May 2002.
- “Seamless Steel Tubes for Pressure Purposes—Technical Delivery Conditions—Part 2: Non-alloy and Alloy Steel Tubes with Specified Elevated Temperature Properties” British Standard BS EN 10216-2:2002+A2:2007:E:1-45, published Aug. 2007.
- “Seamless Steel Tubes for Pressure Purposes—Technical Delivery Conditions—Part 3: Alloy Fine Grain Steel Tubes” British Standard BS EN 10216-3:2002 +A1:2004 E:1-34, published Mar. 2004.
- “Seamless Steel Tubes for Pressure Purposes—Technical Delivery Conditions—Part 4: Non-alloy and Alloy Steel Tubes with Specified Low Temperature Properties” British Standard BS EN 10216-4:2002 +A1:2004 E:1-30, published Mar. 2004.
- Aggarwal, R. K., et al.: “Qualification of Solutions for Improving Fatigue Life at SCR Touch Down Zone”, Deep Offshore Technology Conference, Nov. 8-10, 2005, Vitoria, Espírito Santo, Brazil, in 12 pages.
- Anelli, E., D. Colleluori, M. Pontremoli, G. Cumino, A. Izquierdo, H. Quintanilla, “Metallurgical design of advanced heavy wall seamless pipes for deep-water applications”, 4th International Conference on Pipeline Technology, May 9 to 13, 2004, Ostend, Belgium.
- Asahi, et al., Development of Ultra-high-strength Linepipe, X120, Nippon Steel Technical Report, Jul. 2004, Issue 90, pp. 82-87.
- ASM Handbook, Mechanical Tubing and Cold Finishing, Metals Handbook Desk Edition, (2000), 5 pages.
- Bai M., D. Liu, Y. Lou, X. Mao, L. Li, X. Huo, “Effects of Ti addition on low carbon hot strips produced by CSP process”, Journal of University of Science and Technology Beijing, 2006, vol. 13, N° 3, p. 230.
- Beretta, Stefano et al., “Fatigue Assessment of Tubular Automotive Components in Presence of Inhomogeneities”, Proceedings of IMECE2004, ASME International Mechanical Engineering Congress, Nov. 13-19, 2004, pp. 1-8.
- Berner, Robert A., “Tetragonal Iron Sulfide”, Science, Aug. 31, 1962, vol. 137, Issue 3531, pp. 669.
- Berstein et al., “The Role of Traps in the Microstructural Control of Hydrogen Embrittlement of Steels” Hydrogen Degradation of Ferrous Alloys, Ed. T. Oriani, J. Hirth, and M. Smialowski, Noyes Publications, 1988, pp. 641-685.
- Boulegue, Jacques, “Equilibria in a sulfide rich water from Enghien-les-Bains, France”, Geochimica et Cosmochimica Acta, Pergamon Press, 1977, vol. 41, pp. 1751-1758, Great Britain.
- Bruzzone et al., “Study of Hydrogen Permeation Through Passive Films on Iron Using Electrochemical Impedance Spectroscopy”, PhD Thesis, 2003, Universidad Nacional del Comahue de Buenos Aires, Argentina.
- Cancio et al., “Characterization of microalloy precipitates in the austenitic range of high strength low alloy steels”, Steel Research, 2002, vol. 73, pp. 340-346.
- Carboni, A., A. Pigani, G. Megahed, S. Paul, “Casting and rolling of API X 70 grades for artic application in a thin slab rolling plant”, Stahl u Eisen, 2008, N° 1, p. 131-134.
- Chang, L.C., “Microstructures and reaction kinetics of bainite transformation in Si-rich steels,” XP0024874, Materials Science and Engineering, vol. 368, No. 1-2, Mar. 15, 2004, pp. 175-182, Abstract, Table 1.
- Clark, A. Horrell, “Some Comments on the Composition and Stability Relations of Mackinawite”, Neues Jahrbuch für Mineralogie, 1966, vol. 5, pp. 300-304, London, England.
- Craig, Bruce D., “Effect of Copper on the Protectiveness of Iron Sulfide Films”, Corrosion, National Association of Corrosion Engineers, 1984, vol. 40, Issue 9, pp. 471-474.
- D.O.T. 178.68 Spec. 39, pp. 831-840, Non reusable (non refillable) cylinders, Oct. 1, 2002.
- De Medicis, Rinaldo, “Cubic FeS, A Metastable Iron Sulfide”, Science, American Association for The Advancement of Science, Steenbock Memorial Library, Dec. 11, 1970, vol. 170, Issue 3963, pp. 723-728.
- Echaniz, G., Morales, C., Perez, T., “Advances in Corrosion Control and Materials in Oil and Gas Production” Papers from Eurocorr 97 and Eurocorr 98, 13, P. S. Jackman and L.M. Smith, Published for the European Federation of Corrosion, No. 26, European Federation of Corrosion Publications, 1999.
- European Search Report dated Jun. 18, 2012 of corresponding European Patent Application No. 12154018.1-1215—9 pages.
- Gojic, Mirko and Kosec, Ladislav., “The Susceptibility to the Hydrogen Embrittlement of Low Alloy Cr and CrMo Steels”, ISIJ International, 1997, vol. 37, Issue 4, pp. 412-418.
- Heckmann, et al., Development of low carbon Nb—Ti—B microalloyed steels for high strength large diameter linepipe, Ironmaking and Steelmaking, 2005, vol. 32, Issue 4, pp. 337-341.
- Howells, et al.: “Challenges for Ultra-Deep Water Riser Systems”, IIR, London, Apr. 1997, 11 pages.
- Hutchings et al., “Ratio of Specimen thickness to charging area for reliable hydrogen permeation measurement”, British Corrosion Journal, 1993, vol. 28, Issue 4, pp. 309-312.
- Iino et al., “Aciers pour pipe-lines résistant au cloquage et au criquage dus à l’hydrogène”, Revue de Metallurgie, 1979, vol. 76, Issue 8-9, pp. 591-609.
- Ikeda et al., “Influence of Environmental Conditions and Metallurgical Factors on Hydrogen Induced Cracking of Line Pipe Steel”, Corrosion/80, National Association of Corrosion Engineers, 1980, vol. 8, pp. 8/1-8/18, Houston, Texas.
- Italian Search Report and Written Opinion re IT Application No. IT MI20110179, completed date Aug. 31, 2011, printed date Sep. 2, 2011.
- Johnston, P. W., G. Brooks, “Effect of Al<sub>2</sub>O<sub>3</sub> and TiO<sub>2</sub> Additions on the Lubrication Characteristics of Mould Fluxes”, Molten Slags, Fluxes and Salts '97 Conference, pp. 845-850.
- Prevéy, Paul, et al., “Introduction of Residual Stresses to Enhance Fatigue Performance in the Initial Design”, Proceedings of Turbo Expo 2004, Jun. 14-17, 2004, pp. 1-9.
- Shanabarger, M.R. and Moorhead, R. Dale, “H<sub>2</sub>O Adsorption onto clean oxygen covered iron films”, Surface Science, 1996, vol. 365, pp. 614-624.
- Shoemaker, et al., “Formation of Ferrous Monosulfide Polymorphs During Corrosion of Iron by Aqueous Hydrogen Sulfide at 21 degrees C”, Journal of the Electrochemical Society, 1980, vol. 127, Issue 5, pp. 1007-1015.
- Skoczyłas, G., A. Dasgupta, R. Bommaraju, “Characterization of the chemical interactions during casting of High-titanium low carbon enameling steels”, 1991 Steelmaking Conference Proceeding, pp. 707-717.
- Smyth, D., et al.: Steel Tubular Products, Properties and Selection: Irons, Steels, and High-Performance Alloys, vol. 1, ASM Handbook, ASM International, 1990, p. 327-336.
- Spry, Alan, “Metamorphic Textures”, Pergamon Press, 1969, New York.
- Taira et al., “HIC and SSC Resistance of Line Pipes for Sour Gas Service”, Nippon Kokan Technical Report, 1981, vol. 31, Issue 1-13.
- Taira et al., “Study on the Evaluation of Environmental Condition of Wet Sour Gas”, Corrosion 83 (Reprint. No. 156, National Association of Corrosion Engineers), 1983, pp. 156/2-156/13, Houston, Texas.
- Takeno et al., “Metastable Cubic Iron Sulfide—With Special Reference to Mackinawite”, American Mineralogist, 1970, vol. 55, pp. 1639-1649.
- Tenaris Newsletter for Pipeline Services, Apr. 2005, p. 1-8.
- Tenaris Newsletter for Pipeline Services, May 2003, p. 1-8.
- Thethi, et al.: “Alternative Construction for High Pressure High Temperature Steel Catenary Risers”, OPT USA, Sep. 2003, p. 1-13.
- Thewlis, G., Weldability of X100 linepipe, Science and Technology of Welding and Joining, 2000, vol. 5, Issue 6, pp. 365-377.
- Tivelli, M., G. Cumino, A. Izquierdo, E. Anelli, A. Di Schino, “Metallurgical Aspects of Heavy Wall—High Strength Seamless Pipes for

(56)

**References Cited**

## OTHER PUBLICATIONS

- Deep Water Applications", RioPipeline 2005, Oct. 17 to 19, 2005, Rio (Brasil), Paper n° IBP 1008\_05.
- Todoroki, T. Ishii, K. Mizuno, A. Hongo, "Effect of crystallization behavior of mold flux on slab surface quality of a Ti-bearing Fe—Cr—Ni super alloy cast by means of continuous casting process", Materials Science and Engineering A, 2005, vol. 413-414, p. 121-128.
- Wegst, C.W., "Stahlüssel", Auflage 1989, Seite 119, 2 pages.
- Italian Search Report and Written Opinion re IT Application No. IT MI20110180, completed Sep. 1, 2011, printed date Sep. 2, 2011.
- Fang, Hong-Sheng, et al.: "The Developing Prospect of Air-cooled Bainitic Steels", International Journal of Issi, vol. 2, No. 2, Feb. 1, 2005, pp. 9-18.
- NACE MR0175/ISO 15156-2, Petroleum and Natural Gas Industries—Materials for Use in H<sub>2</sub>S-containing Environments in Oil and Gas Production, Dec. 15, 2003.
- Turconi, G. L.: "Improvement of resistance to SSC initiation and propagation of high strength OCTG through microstructure and precipitation control"; "Paper 01077", NACE International, Houston, TX, Mar. 16, 2001. (XP009141583).
- Vaughan, D. J. and Ridout, M.S., "Moessbauer Studies of Some Sulphide Minerals", J. Inorg Nucl. Chem., 1971, vol. 33, pp. 741-746.
- Izquierdo, et al.: "Qualification of Weldable X65 Grade Riser Sections with Upset Ends to Improve Fatigue Performance of Deepwater Steel Catenary Risers", Proceedings of the Eighteenth International Offshore and Polar Engineering Conference, Vancouver, BC, Canada, Jul. 6-11, 2008, p. 71.
- Johnston, P. W., G.Brooks, "Effect of Al<sub>2</sub>O<sub>3</sub> and TiO<sub>2</sub> Additions on the Lubrication Characteristics of Mould Fluxes", Molten Slags, Fluxes and Salts '97 Conference, pp. 845-850, 1997.
- Keizer, Joel, "Statistical Thermodynamics of Nonequilibrium Processes", Springer-Verlag, 1987.
- Kishi, T., H.Takeucgi, M.Yamamiya, H.Tsuboi, T.Nakano, T.Ando, "Mold Powder Technology for Continuous Casting of Ti-Stabilized Stainless Steels", Nippon Steel Technical Report, No. 34, Jul. 1987, pp. 11-19.
- Korolev, D. F., "The Role of Iron Sulfides in the Accumulation of Molybdenum in Sedimentary Rocks of the Reduced Zone", Geochemistry, 1958, vol. 4, pp. 452-463.
- Lee, Sung Man and Lee, Jai Young, "The Effect of the Interface Character of TiC Particles on Hydrogen Trapping in Steel", Acta Metall., 1987, vol. 35, Issue 11, pp. 2695-2700.
- Mishael, et al., "Practical Applications of Hydrogen Permeation Monitoring," Corrosion, Mar. 28-Apr. 1, 2004, Corrosion 2004, Nacional Association of Corrosion Engineers, vol. Reprint No. 04476.
- Morice et al., "Moessbauer Studies of Iron Sulphides", J. Inorg. Nucl. Chem., 1969, vol. 31, pp. 3797-3802.
- Mukongo, T., P.C.Pistorius, and A.M.Garbers-Craig, "Viscosity Effect of Titanium Pickup by Mould Fluxes for Stainless Steel", Ironmaking and Steelmaking, 2004, vol. 31, No. 2, pp. 135-143.
- Mullet et al., "Surface Chemistry and Structural Properties of Mackinawite Prepared by Reaction of Sulfide Ions with Metallic Iron", Geochemica et Cosmochimica Acta, 2002, vol. 66, Issue 5, pp. 829-836.
- Murcowchick, James B. And Barnes, H.L., "Formation of a cubic FeS", American Mineralogist, 1986, vol. 71, pp. 1243-1246.
- NACE MR0175/ISO 15156-1 Petroleum and natural gas industries—Materials for use in H<sub>2</sub>S-containing Environments in oil and gas production—Part 1: General principles for selection of cracking-resistant materials, Jun. 28, 2007.
- Nagata, M., J. Speer, D. Matlock, "Titanium nitride precipitation behavior in thin slab cast high strength low alloyed steels", Metallurgical and Materials Transactions A, 2002 ,vol. 33A, p. 3099-3110.
- Nakai et al., "Development of Steels Resistant to Hydrogen Induced Cracking in Wet Hydrogen Sulfide Environment", Transactions of the ISIJ, 1979, vol. 19, pp. 401-410.
- Pressure Equipment Directive 97/23/EC, May 29, 1997, downloaded from website:[http://ec.europa.eu/enterprise/pressure\\_equipment/ped/index\\_en.html](http://ec.europa.eu/enterprise/pressure_equipment/ped/index_en.html) on Aug. 4, 2010.
- Prevéey, Paul, et al., "Introduction of Residual Stresses to Enhance Fatigue Performance in the Initial Design", Proceedings of Turbo Expo 2004, Jun. 14-17, 2004, pp. 1-9.
- Rickard, D.T., "The Chemistry of Iron Sulphide Formation at Low Temperatures", Stockholm Contrib. Geol., 1969, vol. 26, pp. 67-95.
- Riecke, Ernst and Bohnenkamp, Konrad, "Über den Einfluss von Gitterserstellen in Eisen auf die Wassersroffdiffusion", Z. Metallkde., 1984, vol. 75, pp. 76-81.

\* cited by examiner



FIG. 1



FIG. 2



FIG. 3



FIG. 4



FIG. 5



FIG. 6



FIG. 7



FIG. 8

## 1

**HEAVY WALL STEEL PIPES WITH  
EXCELLENT TOUGHNESS AT LOW  
TEMPERATURE AND SULFIDE STRESS  
CORROSION CRACKING RESISTANCE**

**CROSS-REFERENCE TO RELATED  
APPLICATIONS**

This application claims priority to Italian Patent Application No. MI2011A000179, entitled "HEAVY WALL STEEL PIPES WITH EXCELLENT TOUGHNESS AT LOW TEMPERATURE AND SULFIDE STRESS CORROSION CRACKING RESISTANCE", filed Feb. 7, 2011. This application is also related to U.S. patent application Ser. No. 13/367,332, entitled "HIGH STRENGTH STEEL PIPES WITH EXCELLENT TOUGHNESS AT LOW TEMPERATURE AND SULFIDE STRESS CORROSION CRACKING RESISTANCE", filed Feb. 6, 2012. The entirety of each of these applications is hereby incorporated by reference and should be considered a part of this specification.

**BACKGROUND**

**1. Field**

Embodiments of the present disclosure relate generally to metal production and, in certain embodiments, relates to methods of producing metallic tubular bars having high toughness at low temperature while concurrently possessing sulfide stress corrosion cracking resistance. Certain embodiments relate to heavy wall seamless steel pipes for risers, line pipes and flow lines for use in the oil and gas industry, including pipes that are suitable for bending.

**2. Description of the Related Art**

Exploration of offshore oil and gas reserves in remote regions of the world is increasingly moving away from conditions where relatively traditional pipe solutions can be utilized and towards more demanding environments. These more demanding environments may incorporate a combination of very challenging factors, including for example, deep water locations, increased pressure and temperature wells, more corrosive products, and lower design temperatures. These conditions, when added to stringent weldability and toughness criteria already associated with pipe specifications for offshore oil and gas exploration applications, place ever increasing demands on the materials and supply capability.

These demands are evident in project developments involving aggressive composition and high operating pressure that require very thick wall, sour service carbon steels. For example, major seamless line pipe manufacturers are able to manufacture pipes of grades X65 and X70 according with American Petroleum Institute (API) 5L and International Organization for Standards (ISO) 3183 standards, with sulfide stress corrosion (SSC) and hydrogen induced cracking (HIC) resistance, when wall thickness (WT) is below 35 mm. However, the conflicting requirements of strength and toughness, combined with the need for sulfide stress corrosion (SSC) and hydrogen induced cracking (HIC) resistance (e.g., sour resistance) in thick wall pipes (e.g., WT greater than or equal to 35 mm) has proven difficult to achieve.

In the complex scenario of line pipe projects for applications such as sour service, deep and ultra-deep water, Arctic-like areas, etc., heavy wall bends have also become an important feature of pipes.

**SUMMARY**

Embodiments of the disclosure are directed to steel pipes or tubes and methods of manufacturing the same. In some

## 2

embodiments, heavy wall, seamless, quenched and tempered (Q&T) steel pipes are provided having a wall thickness (WT) greater than or equal to about 35 mm and a minimum yield strength of about 65 ksi and about 70 ksi, respectively, with excellent low temperature toughness and corrosion resistance (sour service, H<sub>2</sub>S environment). The steel pipes are suitable for use as line pipes and risers, amongst other applications. In some embodiments, the seamless pipes are also suitable to produce bends of the same grade by hot induction bending and off-line quenching and tempering treatment. In one embodiment, the steel pipe has an outside diameter (OD) between about 6" (152 mm) and about 28" (711 mm), and wall thickness (WT) greater than about 35 mm.

In one embodiment, the composition of a seamless, low-alloy steel pipe may comprise (by weight):

about 0.05% to about 0.16% C;  
about 0.20% to about 0.90% Mn;  
about 0.10% to about 0.50% Si;  
about 1.20% to about 2.60% Cr;  
about 0.05% to about 0.50% Ni;  
about 0.80% to about 1.20% Mo;  
about 0.80% W maximum;  
about 0.03% Nb maximum;  
about 0.02% Ti maximum;  
about 0.005% to about 0.12% V;  
about 0.008% to about 0.040% Al;  
about 0.0030% to about 0.012% N;  
about 0.3% Cu maximum;  
about 0.01% S maximum;  
about 0.02% P maximum;  
about 0.001% to about 0.005% Ca;  
about 0.0020% B maximum;  
about 0.020% As maximum;  
about 0.005% Sb maximum;  
about 0.020% Sn maximum;  
about 0.030% Zr maximum;  
about 0.030% Ta maximum;  
about 0.0050% Bi maximum;  
about 0.0030% O maximum; and  
about 0.00030% H maximum;  
with the balance of the composition comprising iron and inevitable impurities.

The steel pipes may be manufactured into different grades. In one embodiment, a 450 MPa (65 ksi) grade steel pipe may be provided with the following properties:

Yield strength (YS): about 450 MPa (65 ksi) minimum and about 600 MPa (87 ksi) maximum.

Ultimate Tensile Strength (UTS): about 535 MPa (78 ksi) minimum and about 760 MPa (110 ksi) maximum.

Elongation, not less than about 20%.

YS/UTS ratio no higher than about 0.91.

In another embodiment, a 485 MPa (70 ksi) grade steel pipe may be provided with the following properties:

Yield strength (YS): about 485 MPa (70 ksi) minimum and about 635 MPa (92 ksi) maximum.

Ultimate Tensile Strength (UTS): about 570 MPa (83 ksi) minimum and about 760 MPa (110 ksi) maximum.

Elongation, not less than about 18%.

YS/UTS ratio no higher than about 0.93.

The steel pipe may have a minimum impact energy of about 200 J/150 J (average/individual) and a minimum average shear area of about 80% for both longitudinal and transverse Charpy V-notch (CVN) tests performed on standard size specimens at about -70° C. according to standard ISO 148-1. Embodiments of the steel pipe may also have a ductile-to-brittle transition temperature, measured by drop weight test

(DWT) according to ASTM 208, lower than about  $-70^{\circ}\text{C}$ . In one embodiment, the steel pipe may have a maximum hardness of about 248 HV10.

Steel pipes manufactured according to embodiments of the present disclosure may exhibit resistance to both hydrogen induced cracking (HIC) and sulfide stress corrosion (SSC) cracking. In one embodiment, discussed in greater detail below, HIC testing performed according with Standard TM0284-2003 Item No. 21215, using NACE solution A and test duration 96 hours, provided the following HIC parameters for the steel pipes when averaged on three sections of three test specimens:

Crack Length Ratio, CLR<5%

Crack Thickness Ratio, CTR=1%

Crack Sensitivity Ratio, CSR=0.2%

In another embodiment, SSC testing of samples of the above described steel pipes was performed in accordance with NACE TM0177, using test solution A and a test duration of about 720 hours. Under these conditions, the steel pipe samples exhibited no apparent failure at about 90% of the specified minimum yield stress (SMYS).

Steel pipes manufactured according to certain embodiments of the disclosure have a microstructure exhibiting substantially no ferrite, substantially no upper bainite, and substantially no granular bainite. The steel pipes may further comprise tempered martensite with volume percentage greater than about 50%, greater than about 60%, preferably greater than about 90%, and most preferably greater than about 95%, as measured according to ASTM E562-08, with tempered lower bainite in a volume percentage less than about 40%, preferably less than about 10%, most preferably less than about 5%. Martensite and bainite, in some embodiments, may be formed at temperatures lower than about  $450^{\circ}\text{C}$ . and about  $540^{\circ}\text{C}$ ., respectively, after re-heating at temperatures of about  $900^{\circ}\text{C}$ . to about  $1060^{\circ}\text{C}$ . for soaking times between about 300 sec to about 3600 sec, and quenching at cooling rates equal or greater than about  $7^{\circ}\text{C./s}$ . In further embodiments, the average prior austenite grain size of the steel pipes, measured according to ASTM Standard E112, is greater than about  $15\text{ }\mu\text{m}$  (lineal intercept) and smaller than about  $100\text{ }\mu\text{m}$ . The average size of regions separated by high angle boundaries (i.e. packet size), in one embodiment, may be smaller than about  $6\text{ }\mu\text{m}$  (preferably smaller than about  $4\text{ }\mu\text{m}$ , most preferably smaller than about  $3\text{ }\mu\text{m}$ ), measured as average lineal intercept on images taken by Scanning Electron Microscopy (SEM) using the Electron Back Scattered Diffraction (EBSD) signal, and considering high-angle boundaries those with misorientation $>45^{\circ}$ . The microstructure may also include presence of one or more precipitates. For example, the microstructure may include precipitates of a first type given by any of MX and  $\text{M}_2\text{X}$ , where M is selected from V, Mo, Nb, and Cr and X is selected from C and N. The size (e.g., average diameter) of the first type of precipitates may be less than about 40 nm. In further embodiments, coarse precipitates of a second type, given by any of  $\text{M}_3\text{C}$ ,  $\text{M}_6\text{C}$ ,  $\text{M}_{23}\text{C}_6$ , may also be present with the fine precipitates of the first type. The average diameter of the second type of precipitates may be between about 80 nm to about 400 nm (precipitates were examined by Transmission Electron Microscopy (TEM) using extraction replica method).

In one embodiment, a steel pipe is provided. The steel pipe comprises a steel composition comprising:

about 0.05 wt. % to about 0.16 wt. % carbon;

about 0.20 wt. % to about 0.90 wt. % manganese;

about 0.10 wt. % to about 0.50 wt. % silicon;

about 1.20 wt. % to about 2.60 wt. % chromium;

about 0.05 wt. % to about 0.50 wt. % nickel;

about 0.80 wt. % to about 1.20 wt. % molybdenum; about 0.005 wt. % to about 0.12 wt. % vanadium; about 0.008 wt. % to about 0.04 wt. % aluminum; about 0.0030 wt. % to about 0.0120 wt. % nitrogen; and about 0.0010 wt. % to about 0.005 wt. % calcium; where the wall thickness of the steel pipe is greater than or equal to about 35 mm; and

where the steel pipe is processed to have a yield strength greater than or equal to about 450 MPa (65 ksi) and where the microstructure of the steel tube comprises martensite in a volume percentage greater than or equal to about 50% and lower bainite in a volume percentage less than or equal to about 50%.

In another embodiment, a method of making a steel pipe is provided. The method comprises providing a steel having a carbon steel composition. The method further comprises forming the steel into a tube having a wall thickness greater than or equal to about 35 mm. The method additionally comprises heating the formed steel tube in a first heating operation to a temperature within the range between about  $900^{\circ}\text{C}$ . to about  $1060^{\circ}\text{C}$ . The method also comprises quenching the formed steel tube at a rate greater than or equal to about  $7^{\circ}\text{C./sec}$ , where the microstructure of the quenched steel is greater than or equal to about 50% martensite and less than or equal to about 50% lower bainite and has an average prior austenite grain size greater than about  $15\text{ }\mu\text{m}$ . The method additionally comprises tempering the quenched steel tube at a temperature within the range between about  $680^{\circ}\text{C}$ . to about  $760^{\circ}\text{C}$ ., where the steel tube, after tempering, has a yield strength greater than about 450 MPa (65 ksi) and a Charpy V-notch energy greater than or equal to about  $150\text{ J/cm}^2$ .

#### BRIEF DESCRIPTION OF THE DRAWINGS

Other features and advantages of the disclosed embodiments will be apparent from the following description taken in connection with the accompanying drawings.

FIG. 1 is a schematic flow diagram illustrating one embodiment of a method for fabricating steel pipes;

FIG. 2 is an embodiment of a continuous cooling transformation (CCT) diagram for an embodiment of a steel of the present disclosure;

FIG. 3 is an optical micrograph illustrating the microstructure of an as-rolled pipe formed according to the disclosed embodiments;

FIG. 4 is an optical micrograph illustrating the microstructure of an as-quenched pipe formed according to the disclosed embodiments;

FIG. 5 is an optical micrograph illustrating austenite grains at about the mid-wall of the as-quenched pipe of FIG. 4;

FIG. 6 is a plot illustrating the intercept distribution of boundaries with misorientation angle greater than about  $45^{\circ}$  for a steel formed according the disclosed embodiments;

FIG. 7 is an optical micrograph at about the mid-wall of the as-quenched pipe bend of Example 2; and

FIG. 8 is an optical micrograph at about the mid-wall of the as-quenched pipe of the comparative example of Example 3.

#### DETAILED DESCRIPTION

Embodiments of the present disclosure provide steel compositions and tubular bars (e.g., pipes) formed using the steel compositions. Respective methods of manufacture are also disclosed. The tubular bars may be employed, for example, as line pipes and risers for use in the oil and gas industry. In certain embodiments, the tubular bars may possess wall thicknesses greater than or equal to about 35 mm and a micro-

structure of martensite and lower bainite without substantial ferrite, upper bainite, or granular bainite. So formed, the tubular bars may possess a minimum yield strength of about 65 ksi and about 70 ksi. In further embodiments, the tubular bars may possess good toughness at low temperatures, as well as resistance to sulfide stress corrosion cracking (SSC) and hydrogen induced cracking (HIC). These properties enable use of the tubular bars in sour service environments. It may be understood, however, that tubular bars comprise one example of articles of manufacture which may be formed from embodiments of the present disclosure and should in no way be construed to limit the applicability of the disclosed embodiments.

The term "bar" as used herein is a broad term and includes its ordinary dictionary meaning and also refers to generally hollow, elongate members which may be straight or have bends or curves and may be formed to a predetermined shape, and any additional forming required to secure the formed tubular bar in an intended location. The bar may be tubular, having a substantially circular outer surface and inner surface, although other shapes and cross-sections are contemplated as well. As used herein, the term "tubular" may refer to any elongate, hollow shape, which need not be circular or cylindrical.

The terms "approximately", "about", and "substantially" as used herein represent an amount equal to or close to a stated amount that still performs a desired function or achieves a desired result. For example, the terms "approximately," "about," and "substantially" may refer to an amount that is within less than 10% of, within less than 5% of, within less than 1% of, within less than 0.1% of, and within less than 0.01% of the stated amount.

The term "room temperature" as used herein has its ordinary meaning as known to those skilled in the art and may include temperatures within the range of about 16° C. (60° F.) to about 32° C. (90° F.).

In general, embodiments of the present disclosure comprise low-alloy carbon steel pipes and methods of manufacture. As discussed in greater detail below, through a combination of steel composition and heat treatment, a steel pipes may be provided having a final microstructure that provides selected mechanical properties of interest, including one or more of minimum yield strength, toughness, hardness, and corrosion resistance in high wall thickness pipes (e.g., WT greater than or equal to about 35 mm).

Embodiments of the disclosed steel compositions may comprise not only carbon (C) but also manganese (Mn), silicon (Si), chromium (Cr), nickel (Ni), molybdenum (Mo), vanadium (V), aluminum (Al), nitrogen (N), and calcium (Ca). Additionally, one or more of the following elements may be optionally present and/or added as well: tungsten (W), niobium (Nb), titanium (Ti), boron (B), zirconium (Zr), and tantalum (Ta). The remainder of the composition may comprise iron (Fe) and impurities. In certain embodiments, the concentration of impurities may be reduced to as low an amount as possible. Embodiments of impurities may include, but are not limited to, copper (Cu), sulfur (S), phosphorous (P), arsenic (As), antimony (Sb), tin (Sn), bismuth (Bi), oxygen (O), and hydrogen (H).

For example, embodiments of the low-alloy steel composition may comprise (in weight % unless otherwise noted):

Carbon within the range between about 0.05% to about 0.16%;

Manganese within the range between about 0.20% to about 0.90%;

Silicon within the range between about 0.10% to about 0.50%;

Chromium within the range between about 1.20% to about 2.60%;

Nickel within the range between about 0.050% to about 0.50%;

5 Molybdenum within the range between about 0.80% to about 1.20%;

Tungsten less than or equal to about 0.80%;

Niobium less than or equal to about 0.030%;

Titanium less than or equal to about 0.020%;

10 Vanadium within the range between about 0.005% to about 0.12%;

Aluminum within the range between about 0.008% to about 0.040%;

15 Nitrogen within the range between about 0.0030% to about 0.012%;

Copper less than or equal to about 0.3%;

Sulfur less than or equal to about 0.01%;

Phosphorous less than or equal to about 0.02%;

Calcium within the range between about 0.001%-0.005%;

Boron less than or equal to about 0.0020%;

Arsenic less than or equal to about 0.020%;

Antimony less than or equal to about 0.005%;

Tin less than or equal to about 0.020%;

Zirconium less than or equal to 0.03%;

Tantalum less than or equal to 0.03%;

Bismuth less than about 0.0050%;

Oxygen less than about 0.0030%;

Hydrogen less than or equal to about 0.00030; and

30 the balance of the composition comprising iron and impurities.

Heat treatment operations performed on pipes formed from the steel composition may include, but are not limited to, quenching and tempering (Q+T). The quenching operation may include reheating a pipe from about room temperature, 35 after hot forming, to a temperature that austenitizes the pipe, followed by a rapid quench. For example, a pipe may be heated to a temperature within the range between about 900° C. to about 1060° C. and held at about the austenitizing temperature for a selected soaking time. Cooling rates during 40 the quench may be selected so as to achieve a selected cooling rate at about the mid-wall of the pipe. For example, pipes may be cooled so as to achieve cooling rates greater than or equal to about 7° C./s at the mid-wall.

Quenching pipes having a WT greater than or equal to 45 about 35 mm and the composition described above may promote the formation of a volume percent of martensite greater than about 50%, preferably greater than about 70% and more preferably greater than about 90% within the pipe. The remaining microstructure of the pipe may comprise lower bainite, with substantially no ferrite, upper bainite, or granular bainite.

Following the quenching operations, pipes may be further subjected to tempering. Tempering may be conducted at a temperature within the range between about 680° C. to about 55 760° C., depending upon the composition of the steel and the target yield strength. In addition to martensite and lower bainite, the microstructure may further exhibit an average prior austenite grain size, measured according to ASTM E112, of about 15  $\mu$ m or about 20  $\mu$ m to about 100  $\mu$ m. The microstructure may also exhibit an average packet size of less than about 6  $\mu$ m. The microstructure may further exhibit one or more precipitates. For example, precipitates of a first type given by any of MX,  $M_2X$ , where M=V, Mo, Nb, or Cr and X=C or N may be present in the microstructure. Precipitates 60 of the first type may have an average diameter less than or equal to about 40 nm. In certain embodiments, precipitates of a second type given by any of  $M_3C$ ,  $M_6C$ , and  $M_{23}C_6$  may be

present. Precipitates of the second type may have an average diameter between about 80 nm to about 400 nm.

In one embodiment, a steel pipe having a WT greater than about 35 mm and the composition and microstructure discussed above may possess the following properties:

Minimum Yield Strength (YS)=about 65 ksi (450 MPa)

Maximum Yield Strength=about 87 ksi (600 MPa)

Minimum Ultimate Tensile Strength (UTS)=about 78 ksi (535 MPa)

Maximum Ultimate Tensile Strength=about 110 ksi (760 MPa)

Elongation at failure=Greater than about 20%

YS/UTS=Less than or equal to about 0.91

In another embodiment, a steel pipe having a WT greater than about 35 mm may be formed having the following properties:

Minimum Yield Strength (YS)=about 70 ksi (485 MPa)

Maximum Yield Strength=about 92 ksi (635 MPa)

Minimum Ultimate Tensile Strength (UTS)=about 83 ksi (570 MPa)

Maximum Ultimate Tensile Strength=about 110 ksi (760 MPa)

Elongation at failure=Greater than about 18%

YS/UTS=Less than or equal to about 0.93

In each of the above embodiments, formed pipe may further exhibit the following impact and hardness properties:

Minimum Impact Energy (Average/Individual at about -70° C.)

=about 200 J/about 150 J

Average Shear Area (CVN at about -70° C.; ISO 148-1)

=about 80% minimum

Ductile-Brittle Transformation Temperature (ASTM E23)

=Less than or equal to about -70° C.

Hardness

=about 248 HV<sub>10</sub> maximum

In each of the above embodiments, formed pipe may further exhibit the following resistance to sulfide stress corrosion (SSC) cracking and hydrogen induced cracking (MC). SSC testing is conducted according to NACE TM 0177 using solution A with a test duration of about 720 hours. HIC testing is conducted according to NACE TM 0284-2003 Item 21215 using NACE solution A and test duration of about 96 hours:

HIC

Crack Length Ratio, CLR=Less than or equal to about 5%

Crack Thickness Ratio, CTR=Less than or equal to about 1%

Crack Sensitivity Ratio, CSR=Less than or equal to about 0.2%

SSC

Failure time at 90% specified minimum yield stress (SMYS)

=Greater than about 720 hours

With reference to FIG. 1, a flow diagram illustrating one embodiment of a method 100 for manufacturing tubular bars is shown. The method 100 includes steel making operations 102, hot forming operations 104, heat treatment operations 106, which may include austenitizing 106A, quenching 106B, tempering 106C, and finishing operations 110. It may be understood that the method 100 may include greater or fewer operations and the operations may be performed in a different order than that illustrated in FIG. 1, as necessary.

Operation 102 of the method 100 preferably comprises fabrication of the steel and production of a solid metal billet capable of being pierced and rolled to form a metallic tubular bar. In further embodiments, selected steel scrap, cast iron, and sponge iron may be employed to prepare the raw material for the steel composition. It may be understood, however, that

other sources of iron and/or steel may be employed for preparation of the steel composition.

Primary steelmaking may be performed using an electric arc furnace to melt the steel, decrease phosphorous and other impurities, and achieve a selected temperature. Tapping and deoxidation, as well as addition of alloying elements may be further performed.

One of the main objectives of the steelmaking process is to refine the iron by removal of impurities. In particular, sulfur and phosphorous are prejudicial for steel because they degrade the mechanical properties of the steel. In one embodiment, secondary steelmaking may be performed in a ladle furnace and trimming station after primary steelmaking to perform specific purification steps.

During these operations, very low sulfur contents may be achieved within the steel, calcium inclusion treatment is performed, and inclusion flotation is performed. In one embodiment inclusion flotation may be performed by bubbling inert gases in the ladle furnace to force inclusions and impurities to float. This technique produces a fluid slag capable of absorbing impurities and inclusions. In this manner, a high quality steel having the desired composition with a low inclusion content may be provided.

Table 1 illustrates embodiments of the steel composition, in weight percent (wt. %) unless otherwise noted.

TABLE 1

| Element | Steel composition ranges |                |                |                |                |                |
|---------|--------------------------|----------------|----------------|----------------|----------------|----------------|
|         | Composition Range        |                |                |                |                |                |
|         | General                  | More Preferred | More Preferred | Most Preferred | Most Preferred | Most Preferred |
| C       | 0.05                     | 0.16           | 0.07           | 0.14           | 0.08           | 0.12           |
| Mn      | 0.20                     | 0.90           | 0.30           | 0.60           | 0.30           | 0.50           |
| Si      | 0.10                     | 0.50           | 0.10           | 0.40           | 0.10           | 0.25           |
| Cr      | 1.20                     | 2.60           | 1.80           | 2.50           | 2.10           | 2.40           |
| Ni      | 0.05                     | 0.50           | 0.05           | 0.20           | 0.05           | 0.20           |
| Mo      | 0.80                     | 1.20           | 0.90           | 1.10           | 0.95           | 1.10           |
| W       | 0.00                     | 0.80           | 0.00           | 0.60           | 0.00           | 0.30           |
| Nb      | 0.000                    | 0.030          | 0.000          | 0.015          | 0.000          | 0.010          |
| Ti      | 0.000                    | 0.020          | 0.000          | 0.010          | 0.000          | 0.010          |
| V       | 0.005                    | 0.12           | 0.050          | 0.10           | 0.050          | 0.07           |
| Al      | 0.008                    | 0.040          | 0.010          | 0.030          | 0.015          | 0.025          |
| N       | 0.0030                   | 0.0120         | 0.0030         | 0.0100         | 0.0030         | 0.0080         |
| Cu      | 0.00                     | 0.30           | 0.00           | 0.20           | 0.00           | 0.15           |
| S       | 0.000                    | 0.010          | 0.000          | 0.005          | 0.000          | 0.003          |
| P       | 0.000                    | 0.020          | 0.000          | 0.012          | 0.000          | 0.010          |
| Ca      | 0.0010                   | 0.0050         | 0.0010         | 0.0030         | 0.0015         | 0.0030         |
| B       | 0.0000                   | 0.0020         | 0.0005         | 0.0012         | 0.0008         | 0.0014         |
| As      | 0.000                    | 0.020          | 0.000          | 0.015          | 0.000          | 0.015          |
| Sb      | 0.0000                   | 0.0050         | 0.0000         | 0.0050         | 0.0000         | 0.0050         |
| Sn      | 0.000                    | 0.020          | 0.000          | 0.015          | 0.000          | 0.015          |
| Zr      | 0.000                    | 0.030          | 0.000          | 0.015          | 0.000          | 0.010          |
| Ta      | 0.000                    | 0.030          | 0.000          | 0.015          | 0.000          | 0.010          |
| Bi      | 0.0000                   | 0.0050         | 0.0000         | 0.0050         | 0.0000         | 0.0050         |
| O       | 0.000                    | 0.0030         | 0.000          | 0.0020         | 0.000          | 0.0015         |
| H       | 0.0000                   | 0.00030        | 0.0000         | 0.00025        | 0.0            | 0.00020        |

Carbon (C) is an element whose addition to the steel composition may inexpensively raise the strength of the steel and refine the microstructure, reducing the transformation temperatures. In an embodiment, if the C content of the steel composition is less than about 0.05%, it may be difficult in some embodiments to obtain the strength desired in articles of manufacture, particularly tubular products. On the other hand, in other embodiments, if the steel composition has a C content greater than about 0.16%, in some embodiments, toughness is impaired, and weldability may decrease, making

more difficult and expensive any welding process if joining is not performed by thread joints. In addition, the risk of developing quenching cracks in steels with high hardenability increases with the carbon content. Therefore, in an embodiment, the C content of the steel composition may be selected within the range between about 0.05% to about 0.16%, preferably within the range between about 0.07% to about 0.14%, and more preferably within the range between about 0.08% to about 0.12%.

Manganese (Mn) is an element whose addition to the steel composition may be effective in increasing the hardenability, strength and toughness of the steel. In an embodiment, if the Mn content of the steel composition is less than about 0.20% it may be difficult in some embodiments to obtain the desired strength in the steel. However, in another embodiment, if the Mn content of the steel composition exceeds about 0.90%, in some embodiments banding structures may become marked in some embodiments, and toughness and HIC/SSC resistance may decrease. Therefore, in an embodiment, the Mn content of the steel composition may be selected within the range between about 0.20% to about 0.90%, preferably within the range between about 0.30% to about 0.60%, and more preferably within the range between about 0.30% to about 0.50%.

Silicon (Si) is an element whose addition to the steel composition may have a deoxidizing effect during steel making process and may also raise the strength of the steel (e.g., solid solution strengthening). In an embodiment, if the Si content of the steel composition is less than about 0.10%, the steel in some embodiments may be poorly deoxidized during steel-making process and exhibit a high level of micro-inclusions. In another embodiment, if the Si content of the steel composition exceeds about 0.50%, both toughness and formability of the steel may decrease in some embodiments. Si content higher than about 0.5% are also recognized to have a detrimental effect on surface quality when the steel is processed at high temperatures (e.g., temperatures greater than about 1000° C.) in oxidizing atmospheres, because surface oxide (scale) adherence is increased due to fayalite formation and the risk of surface defect is higher. Therefore, in an embodiment, the Si content of the steel composition may be selected within the range between about 0.10% to about 0.50%, preferably within the range between about 0.10% to about 0.40%, and more preferably within the range between about 0.10% to about 0.25%.

Chromium (Cr) is an element whose addition to the steel composition may increase hardenability, decrease transformation temperatures, and increase tempering resistance of the steel. Therefore the addition of Cr to steel compositions may be desirable for achieving high strength and toughness levels. In an embodiment, if the Cr content of the steel composition is less than about 1.2%, it may be difficult to obtain the desired strength and toughness, some embodiments. In another embodiment, if the Cr content of the steel composition exceeds about 2.6%, the cost may be excessive and toughness may decrease due to enhanced precipitation of coarse carbides at grain boundaries, in some embodiments. In addition, weldability of the resultant steel may be reduced, making the welding process more difficult and expensive, if joining is not performed by thread joints. Therefore, in an embodiment, the Cr content of the steel composition may be selected within the range between about 1.2% to about 2.6%, preferably within the range between about 1.8% to about 2.5%, and more preferably within the range between about 2.1% to about 2.4%.

Nickel (Ni) is an element whose addition may increase the strength and toughness of the steel. However, in an embodiment, when Ni addition exceeds about 0.5%, a negative effect on scale adherence has been observed, with higher risk of surface defect formation. Also, in other embodiments, Ni contents higher than about 1% are recognized to have a detrimental effect on sulfide stress corrosion cracking. Therefore, in an embodiment, the Ni content of the steel composition may be selected within the range between about 0.05% to about 0.5%.

Molybdenum (Mo) is an element whose addition to the steel composition may improve hardenability and hardening by solid solution and fine precipitation. Mo may assist in retarding softening during tempering, promoting the formation of very fine MC and M<sub>2</sub>C precipitates. These particles may be substantially uniformly distributed in the matrix and may also act as beneficial hydrogen traps, slowing down the atomic hydrogen diffusion towards the dangerous traps, usually at grain boundaries, which behave as crack nucleation sites. Mo also reduces the segregation of phosphorous to grain boundaries, improving resistance to inter-granular fracture, with beneficial effects also on SSC resistance because high strength steels which suffer hydrogen embrittlement exhibit an intergranular fracture morphology. Therefore, by increasing the Mo content of the steel composition, the desired strength can be achieved at higher tempering temperatures, which promote better toughness levels. In an embodiment, in order to exert the effect thereof, the Mo content may be greater than or equal to about 0.80%. However, in other embodiments, for Mo contents higher than about 1.2% a saturation effect on hardenability is noted and weldability may be reduced. As Mo ferroalloy is expensive, in an embodiment, the Mo content of the steel composition may be selected within the range between about 0.8 to about 1.2%, preferably within the range between about 0.9% to about 1.1%, and more preferably within the range between about 0.95% to about 1.1%.

Tungsten (W) is an element whose addition to the steel composition is optional and may increase the strength at room and elevated temperatures by forming tungsten carbide which develops secondary hardening. W is preferably added when the steel use is required at high temperatures. The behavior of W is similar to that of Mo in terms of hardenability but its effectiveness is about one half of that of Mo. Tungsten reduces the steel oxidation and, as a result, less scale is formed during reheating processes at high temperatures. However, as its cost is very high, in an embodiment, the W content of the steel composition may be selected to be less than or equal to about 0.8%.

Niobium (Nb) is an element whose addition to the steel composition is optional and may be provided to form carbides and nitrides and may be further used to refine the austenitic grain size during hot rolling and re-heating before quenching. However Nb is not needed in embodiments of present steel composition to refine the austenite grains as a predominant martensite structure is formed and a fine packet is formed even in the case of coarse austenite grains when low transformation temperatures are promoted through a proper balance of other chemical elements such as Cr, Mo, and C.

Nb precipitates as carbonitride may increase the steel strength by particle dispersion hardening. These fine and round particles may be substantially uniformly distributed in the matrix and also act as hydrogen traps, beneficially slowing down the atomic hydrogen diffusion towards the dangerous traps, usually at grain boundaries, which behave as crack nucleation sites. In an embodiment, if the Nb content is higher than about 0.030%, a coarse precipitate distribution that impair toughness may be formed. Therefore, in an embodiment, the Nb content of the steel composition may be selected

## 11

to be less than or equal to about 0.030%, preferably less than or equal to about 0.015%, and more preferably less than or equal to about 0.01%.

Titanium (Ti) is an element whose addition to the steel composition is optional and may be provided to refine austenitic grain size in high temperature processes, forming nitrides and carbonitrides. However it is not needed in embodiments of present steel composition, except when it is used to protect boron that remains in solid solution improving hardenability, especially in the case of pipes with wall thickness greater than about 25 mm. For example, Ti binds nitrogen and avoids BN formation). Additionally, in certain embodiments, when Ti is present in concentrations higher than about 0.02%, coarse TiN particles may be formed that impair toughness. Accordingly, in an embodiment, the Ti content of the steel composition may be less than or equal to about 0.02%, and more preferably less than or equal to about 0.01% when boron is below about 0.0010%.

Vanadium (V) is an element whose addition to the steel composition may increase strength by carbonitride precipitation during tempering. These fine and round particles may also be substantially uniformly distributed within the matrix and act as beneficial hydrogen traps. In an embodiment, if the V content is less than about 0.05%, it may be in some embodiments difficult to obtain the desired strength. However, in another embodiment, if the V content is higher than 0.12%, a large volume fraction of vanadium carbide particles may be formed with subsequent reduction in toughness. Therefore, in certain embodiments, the Nb content of the steel composition may be selected to be less than or equal to about 0.12%, preferably within the range between about 0.05% to about 0.10%, and more preferably within the range between about 0.05% to about 0.07%.

Aluminum (Al) is an element whose addition to the steel composition has a deoxidizing effect during steel making process and may refine the steel grain. In an embodiment, if the Al content of the steel composition is higher than about 0.040%, coarse precipitates of AlN that impair toughness and/or Al-rich oxides (e.g., non-metallic inclusions) that impair HIC and SSC resistance may be formed. Accordingly, in an embodiment, the Al content of the steel may be selected to be less than or equal to about 0.04%, preferably less than or equal to about 0.03%, and more preferably less than or equal to about 0.025%.

Nitrogen (N) is an element whose content within the steel composition is preferably selected to be greater than or equal to about 0.0030%, in one embodiment, in order to form carbonitrides of V, Nb, Mo and Ti. However, in other embodiments, if the N content of the steel composition exceeds about 0.0120%, the toughness of the steel may be degraded. Therefore, the N content of the steel composition may be selected within the range between about 0.0030% to about 0.0120%, preferably within the range between about 0.0030% to about 0.0100%, and more preferably within the range between about 0.0030% to about 0.0080%.

Copper (Cu) is an impurity element that is not needed in embodiments of the steel composition. However, depending on the manufacturing process, the presence of Cu may be unavoidable. Therefore, the Cu content may be limited to as low as possible. For example, in an embodiment, the Cu content of the steel composition may be less than or equal to about 0.3%, preferably less than or equal to about 0.20%, and more preferably less than or equal to about 0.15%.

Sulfur (S) is an impurity element that may decrease both toughness and workability of the steel, as well as HIC/SSC resistance. Accordingly, the S content of the steel in some embodiments may be kept as low as possible. For example, in

## 12

an embodiment, the Cu content of the steel composition may be less than or equal to about 0.01%, preferably less than or equal to about 0.005%, and more preferably less than or equal to about 0.003%.

5 Phosphorous (P) is an impurity element that may cause the toughness and HIC/SSC resistance of high strength steel to decrease. Accordingly, the P content in some embodiments may be kept as low as possible. For example, in an embodiment, the P content of the steel composition may be less than or equal to about 0.02%, preferably less than or equal to about 0.012%, and more preferably less than or equal to about 0.010%.

15 Calcium (Ca) is an element whose addition to the steel composition may assist with control of the shape of inclusions and enhancement of the HIC resistance by forming fine and substantially round sulfides. In an embodiment, in order to provide these benefits, the Ca content of the steel composition may be selected to be greater than or equal to about 0.0010% when the sulfur content of the steel composition is 20 higher than about 0.0020%. However in other embodiments, if the Ca content of the steel composition exceeds about 0.0050% the effect of the Ca addition may be saturated and the risk of forming clusters of Ca-rich non-metallic inclusions 25 that reduce HIC and SSC resistance may be increased. Accordingly, in certain embodiments, the maximum Ca content of the steel composition may be selected to be less than or equal to about 0.0050%, and more preferably less than or equal to about 0.0030%, while the minimum Ca content may 30 be selected to be greater than or equal to about 0.0010%, and most preferably to greater than or equal to about 0.0015%.

35 Boron (B) is an element whose addition to the steel composition is optional and may be provided for improving the hardenability of the steel. B can be used for inhibiting ferrite formation. In an embodiment, the lower limit of the B content of the steel composition to provide these beneficial effects may be about 0.0005%, while the beneficial effects may be saturated with boron contents higher than about 0.0020%. Therefore, in selected embodiments, the maximum B content 40 of the steel composition may be selected to be less than or equal to about 0.0020%.

45 Arsenic (As), tin (Sn), antimony (Sb) and bismuth (Bi) are impurity elements that are not needed in embodiments of the steel composition. However, depending on the manufacturing process, the presence of these impurity elements may be unavoidable. Therefore, the As and Sn contents within the steel composition may be selected to be less than or equal to about 0.020%, and more preferably less than or equal to about 0.015%. The Sb and Bi contents may be selected to be less 50 than or equal to about 0.0050%.

55 Zirconium (Zr) and tantalum (Ta) are elements that act as strong carbide and nitride formers, similar to Nb and Ti. These elements may be optionally added to the steel composition, as they are not needed in embodiments of present steel composition to refine the austenite grains. Zr and Ta fine carbonitrides may increase the steel strength by particle dispersion hardening and may also act as beneficial hydrogen traps, slowing down the atomic hydrogen diffusion towards the dangerous traps. In an embodiment, if the Zr or Ta content 60 is greater than or equal to about 0.030%, a coarse precipitate distribution that may impair toughness of the steel may be formed. Zirconium may also act as a deoxidizing element in steel and combine with the sulfur. However, as addition to steel in order to promote globular non-metallic inclusions, in certain embodiments, Ca may be preferred over Zr. Therefore, the content of Zr and Ta within the steel composition 65 may be selected to be less than or equal to about 0.03%.

The total oxygen (O) content of the steel composition is the sum of the soluble oxygen and the oxygen in the non-metallic inclusions (oxides). As it is practically the oxygen content in the oxides in a well deoxidized steel, an oxygen content that is too high means a high volume fraction of non-metallic inclusions and less resistance to HIC and SSC. Accordingly, in an embodiment, the oxygen content of the steel may be selected to be less than or equal to about 0.0030%, preferably less than or equal to about 0.0020%, and more preferably less than or equal to about 0.0015%.

Following the production of the fluid slag having a composition as described above, the steel may be cast into a round solid billet having a substantially uniform diameter along the steel axis. For example, round billets having a diameter within the range between about 330 mm to about 420 mm may be produced in this manner.

The billet thus fabricated may be formed into a tubular bar through hot forming processes 104. In an embodiment, a solid, cylindrical billet of clean steel may be heated to a temperature of about 1200° C. to 1,340° C., preferably about 1280° C. For example, the billet may be reheated by a rotary hearth furnace. The billet may be further subject to a rolling mill. Within the rolling mill, the billet may be pierced, in certain preferred embodiments utilizing the Manessmann process, and hot rolling is used to substantially reduce the outside diameter and wall thickness of the tube, while the length is substantially increased. In certain embodiments, the Manessmann process may be performed at temperatures within the range between about 1200° C. to about 1280° C. The obtained hollow bars may be further hot rolled at temperatures within the range between about 1000° C. to about 1200° C. in a retained mandrel continuous mill. Accurate sizing may be carried out by a sizing mill and the seamless tubes cooled in air to about room temperature in a cooling bed. For example, pipes with outer diameters (OD) within the range between about 6 inches to about 16 inches may be formed in this manner.

After rolling the pipes may be in-line heated, without cooling at room temperature, by an intermediate furnace for making temperature more uniform, and accurate sizing may be carried out by a sizing mill. Subsequently, the seamless pipes may be cooled in air down to room temperature in a cooling bed. In the case of a pipe having a final OD greater than about 16 inches, the pipes produced by the medium size mill may be processed by a rotary expansion mill. For example, medium size pipes may be reheated by a walking beam furnace to a temperature within the range between about 1150° C. to about 1250° C., expanded to the desired diameter by the expander mill at a temperature within the range between about 1100° C. to about 1200° C., and in-line reheated before final sizing.

In a non-limiting example, a solid bar may be hot formed as discussed above into a tube possessing an outer diameter within the range between about 6 inches to about 16 inches and a wall thickness greater than about 35 mm.

The final microstructure of the formed pipe may be determined by the composition of the steel provided in operation 102 and heat treatments performed in operations 106. The composition and microstructure, in turn, may give rise to the properties of the formed pipe.

In one embodiment, promotion of martensite formation may refine the packet size (the size of the regions separated by high-angle boundaries that offer higher resistance to crack propagation; the higher the misorientation, the higher the energy a crack requires to cross the boundary) and improve the toughness of the steel pipe for a given yield strength. Increasing the amount of martensite in as-quenched pipes may further allow the use of higher tempering temperatures

for a given strength level. Therefore, in an embodiment, it is a goal of the method to achieve a predominantly martensitic microstructure at relatively low temperatures (e.g., transformation of austenite at temperatures less than or equal to about 450° C. In an embodiment, the martensitic microstructure may comprise a volume percent of martensite greater than or equal to about 50%. In further embodiments, the volume percent of martensite may be greater than or equal to about 70%. In further embodiments, the volume percent of martensite may be greater than or equal to about 90%.

In another embodiment, hardenability of the steel, the relative ability of the steel to form martensite when quenched, may be improved through the composition and microstructure. In one aspect, addition of elements such as Cr and Mo are effective in reducing the transformation temperature of martensite and bainite and increase the resistance to tempering. Beneficially, a higher tempering temperature may then be used to achieve a given strength level (e.g., yield strength). In another aspect, a relatively coarse prior austenite grain size (e.g., about 15 or 20  $\mu\text{m}$  to about 100  $\mu\text{m}$ ) may improve hardenability.

In a further embodiment, the sulfide stress corrosion cracking (SSC) resistance of the steel may be improved through the composition and microstructure. In one aspect, the SSC may be improved by increased content of martensite within the pipe. In another aspect, tempering at very high temperatures may improve the SSC of the pipe, as discussed in greater detail below.

In order to promote martensite formation at temperatures less than or equal to about 450° C., the steel composition may further satisfy Equation 1, where the amounts of each element are given in wt. %:

$$60\text{C \%} + \text{Mo \%} + 1.7\text{Cr \%} > 10 \quad \text{Eq. 1}$$

If a significant amount of bainite (e.g., less than about 50 volume %) is present after quenching, the temperature at which the bainite forms should be less than or equal to about 540° C. in order to promote a relatively fine packet, with substantially no upper bainite or granular bainite (a mixture of bainitic dislocated-ferrite and islands of high C martensite and retained austenite).

In order to promote the bainite formation at a temperature less than or equal to about 540° C. (e.g., lower bainite), the steel composition may additionally satisfy Equation 2, where the amounts of each element are given in wt. %:

$$60\text{C \%} + 41\text{Mo \%} + 34\text{Cr \%} > 70 \quad \text{Eq. 2}$$

FIG. 2 illustrates a Continuous Cooling Transformation (CCT) diagram of a steel with composition within the claimed ranges generated by dilatometry. FIG. 2 clearly indicates that, even in the case of high Cr and Mo contents, in order to substantially avoid the formation of ferrite and have an amount of martensite greater than or equal to about 50% in volume, an average austenite grain size (AGS) greater than about 20  $\mu\text{m}$  and a cooling rate greater than about 7° C./s. may be employed.

Notably, normalizing (e.g., austenitizing followed by cooling in still air), may not achieve the desired martensite microstructure because the typical average cooling rates between about 800° C. and 500° C. for pipes of wall thickness between about 35 mm and about 60 mm is lower than about 1° C./s. Water quenching may be employed to achieve the desired cooling rates at about the pipe mid-wall and form martensite and lower bainite at temperatures lower than about 450° C. and about 540° C., respectively. Therefore, the as-rolled pipes may be reheated in a furnace and water quenched in quenching operation 106A after air-cooling from hot rolling.

For example, in one embodiment of the austenitizing operations 106A, the temperatures of the zones of the furnace may be selected in order to allow the pipe to achieve the target austenitizing temperature with a tolerance lower than about  $\pm 20^\circ\text{C}$ . Target austenitizing temperatures may be selected within the range between about  $900^\circ\text{C}$ . to about  $1060^\circ\text{C}$ . The heating rate may be selected within the range between about  $0.1^\circ\text{C./s}$  to about  $0.2^\circ\text{C./s}$ . The soaking time, the time from when the pipe achieves the final target temperature minus about  $10^\circ\text{C}$ . and the exit from the furnace, may be selected within the range between about 300 sec to about 1800 sec. Austenitizing temperatures and holding times may be selected depending on chemical composition, wall thickness, and desired austenite grain size. At the exit of the furnace, the pipe may be descaled to remove the surface oxide and is rapidly moved to a water quenching system.

In the quenching operations 106B, external and internal cooling may be employed to achieve the desired cooling rates at about the mid-wall of the pipe (e.g., greater than about  $7^\circ\text{C./s}$ ). As discussed above, cooling rates within this range may promote the formation of a volume percent of martensite greater than about 50%, preferably greater than about 70%, and more preferably greater than about 90%. The remaining microstructure may comprise lower bainite, (i.e. bainite formed at temperatures lower than about  $540^\circ\text{C}$ . with a typical morphology including fine precipitation within the bainite laths, without coarse precipitates at lath boundaries as in the case of upper bainite, which is usually formed at temperatures higher than about  $540^\circ\text{C}$ .).

In one embodiment, the water quench of quenching operations 106B may be performed by dipping the pipe in a tank containing stirred water. The pipe may be rapidly rotated during quenching to make the heat transfer high and uniform and avoid pipe distortion. Additionally, in order to remove the steam developed inside the pipe, an inner water jet may also be employed. In certain embodiments, the water temperature may not be higher than about  $40^\circ\text{C}$ ., preferably less than about  $30^\circ\text{C}$ . during quenching operations 106B.

After quenching operations 106B, the pipe may be introduced in another furnace for the tempering operations 106C. In certain embodiments, the tempering temperature may be selected to be sufficiently high so as to produce a relatively low dislocation density matrix and more carbides with a substantially round shape (i.e., a higher degree of spheroidization). This spheroidization improves the impact toughness of the pipes, as needle shaped carbides at lath and grain boundaries may provide easier crack paths.

Tempering the martensite at temperatures sufficiently high to produce more spherical, dispersed carbides may promote trans-granular cracking and better SSC resistance. Crack propagation may be slower in steels that possess a high number of hydrogen trapping sites and fine, dispersed precipitates having spherical morphologies give better results.

By forming a microstructure including tempered martensite, as opposed to a banded microstructure (e.g., ferrite-pearlite or ferrite-bainite), the HIC resistance of the steel pipe may be further increased.

In one embodiment, the tempering temperature may be selected within the range between about  $680^\circ\text{C}$ . to about  $760^\circ\text{C}$ . depending on the chemical composition of the steel and the target yield strength. The tolerances for the selected tempering temperature may be within the range of about  $\pm 15^\circ\text{C}$ . The pipe may be heated at a rate between about  $0.1^\circ\text{C./s}$  to about  $0.2^\circ\text{C./s}$  to the selected tempering temperature. The pipe may be further held at the selected tempering temperature for a duration of time selected within the range between about 1800 sec to about 5400 sec.

Notably, the packet size is not significantly influenced by the tempering operations 106C. However, packet size may decrease with a reduction of the temperature at which austenite transforms. In traditional low-carbon steels with carbon equivalents lower than about 0.43%, tempered bainite may show a coarser packet size (e.g., about  $7\text{ }\mu\text{m}$  to about  $12\text{ }\mu\text{m}$ ) as compared with that of the tempered martensite within the instant application (e.g. less than or equal to about  $6\text{ }\mu\text{m}$ , such as from within the range about  $6\text{ }\mu\text{m}$  to about  $2\text{ }\mu\text{m}$ ).

10 The martensite packet size is nearly independent of the average austenite grain size and may remain fine (e.g., an average size less than or equal to about  $6\text{ }\mu\text{m}$ ) even in the case of relatively coarse average austenite grain size (e.g., about  $15\text{ }\mu\text{m}$  or about  $20\text{ }\mu\text{m}$  to about  $100\text{ }\mu\text{m}$ ).

15 Finishing operations 110 may include, but are not limited to, straightening and bending operations. Straightening may be performed at temperatures below the tempering temperature and above about  $450^\circ\text{C}$ .

20 In one embodiment, bending may be performed by hot induction bending. Hot induction bending is a hot deformation process which concentrates in a narrow zone, referred to as hot tape, that is defined by an induction coil (e.g., a heating ring) and a quenching ring that sprays water on the external surface of the structure to be bent. A straight (mother) pipe is 25 pushed from its back, while the front of the pipe is clamped to an arm constrained to describe a circular path. This constraint provokes a bending moment on the entire structure, but the pipe is plastically deformed substantially only within correspondence of the hot tape. The quenching ring plays therefore 30 two simultaneous roles: (i) to define the zone under plastic deformation and (ii) to in-line quench the hot bend.

The diameter of both heating and quenching rings is about 20 mm to about 60 mm larger than the outside diameter (OD) of the mother pipe. The bending temperature at both exterior 35 and interior surfaces of the pipe may be continuously measured by pyrometers.

In conventional pipe fabrication, the bends may be subjected to a stress relieving treatment after bending and quenching by a tempering treatment at a relatively low temperature to achieve the final mechanical properties. However, 40 it is recognized that the in-line quenching and tempering operations performed during finishing operations 110 may produce a microstructure that is different than that obtained from the off-line quenching and tempering operations 106B, 45 106C. Therefore, in an embodiment of the disclosure, as discussed above in operations 106B, 106C, in order to substantially regenerate the microstructure obtained after operations 106B, 106C. Therefore, the bends may, be reheated in a furnace and then rapidly immersed into a quenching tank with stirred water and then tempered in a furnace.

In an embodiment, the temper after bending may be performed at a temperature within the range between about  $710^\circ\text{C}$ . to about  $760^\circ\text{C}$ . The pipe may be heated at a rate within the 55 range between about  $0.05\text{ C/s}$  to about  $0.2^\circ\text{C./s}$ . A hold time within the range between about 1800 sec to about 5400 sec may be employed after the target tempering temperature has been achieved.

FIG. 3 is an optical micrograph (2% nital etching) illustrating the microstructure of an as-rolled pipe formed according to the disclosed embodiments. The composition of the pipe was 0.14% C, 0.46% Mn, 0.24% Si, 2.14% Cr, 0.95% Mo, 0.11% Ni, 0.05% V<0.01%, 0.014% Al, 0.007% N, 0.0013% Ca, 0.011% P, 0.001% S, 0.13% Cu. The pipe possessed an outer diameter (OD) of about 273 mm and a wall thickness of about 44 mm. As illustrated in FIG. 3, the as-rolled pipe exhibits a microstructure that is mainly bainite and some ferrite at the prior austenite boundaries. The average

austenite grain size (AGS) of the as-rolled pipe, measured according to ASTM E112 as lineal intercept, was approximately 102.4  $\mu\text{m}$ .

FIG. 4 is an optical micrograph illustrating the microstructure of the pipe after quenching according to the disclosed embodiments. As illustrated in FIG. 4, the as-quenched pipe exhibits a microstructure that is martensite with a volume percentage greater than 50% (measured according to ASTM E562-08) and lower bainite with a volume percentage less than about 40%. The microstructure does not substantially include ferrite, upper bainite, or granular bainite (a mixture of bainite dislocated-ferrite and islands of high C martensite and retained austenite).

FIG. 5 is an optical micrograph illustrating the mid-wall of the as-quenched pipe of FIG. 4. Selective etching is performed to reveal prior austenite grain boundaries of the as-quenched pipe and determined the prior austenite grain size to be approximately 47.8  $\mu\text{m}$ .

Even when the austenite grain is coarse, as it is in this instance, the packet size of the steel after quenching and tempering may be maintained below approximately 6  $\mu\text{m}$  if a predominant martensite structure (e.g., martensite greater than about 50% in volume) is formed and lower bainite forms at relatively low temperatures (<540° C.).

Packet size is measured as average lineal intercept on images taken by Scanning Electron Microscopy (SEM) using the Electron Back Scattered Diffraction (EBSD) signal, and considering high-angle boundaries those with misorientation greater than about 45°. Measurement by the lineal intercept method gave distribution shown in FIG. 6, with an average the packet size value of about 5.8  $\mu\text{m}$  although the prior austenite grain size had an average value of about 47.8  $\mu\text{m}$ .

On the quenched and tempered pipe, fine precipitates of a first type given by any of MX, M<sub>2</sub>X, where M is Mo or Cr or V, Nb, Ti when present, and X is C or N, with size (e.g., average diameter) less than about 40 nm were also detected by Transmission Electron Microscopy (TEM), in addition to coarse precipitates of the type M<sub>3</sub>C, M<sub>6</sub>C, M<sub>23</sub>C<sub>6</sub> with an average diameter within the range between about 80 nm to about 400 nm.

cussed above. Corresponding mechanical properties, including yield and tensile strengths, hardness, elongation, toughness, and HIC/SSC resistance are further discussed.

5

### Example 1

#### Mechanical and Microstructural Properties of Quenched and Tempered Thick-Wall Pipes

10 The microstructural and mechanical properties of the steel of Table 2 were investigated. With respect to the measurement of microstructural parameters, austenite grain size (AGS) was measured in accordance with ASTM E112, packet size was measured using an average lineal intercept on images taken by scanning electron microscopy (SEM) using the electron backscatter diffraction (EBSD) signal, the volume of martensite was measured in accordance with ASTM E562, the volume of lower bainite was measured in accordance with ASTM E562, the volume percentage of non-metallic inclusions was measured by automatic image analysis using optical microscopy in accordance with ASTM E1245, and the presence of precipitates was investigated by transmission electron microscopy (TEM) using the extraction replica method.

15 20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880 9885 9890 9895 9900 9905 9910 9915 9920 9925 9930 9935 9940 9945 9950 9955 9960 9965 9970 9975 9980 9985 9990 9995 10000 10005 10010 10015 10020 10025 10030 10035 10040 10045 10050 10055 10060 10065 10070 10075 10080 10085 10090 10095 10100 10105 10110 10115 10120 10125 10130 10135 10140 10145 10150 10155 10160 10165 10170 10175 10180 10185 10190 10195 10200 10205 10210 10215 10220 10225 1023

TABLE 3

| Chemical composition of seamless pipes of example 1 |       |        |      |       |       |        |       |        |        |       |       |  |
|-----------------------------------------------------|-------|--------|------|-------|-------|--------|-------|--------|--------|-------|-------|--|
| Pipe                                                | C     | Mn     | Si   | P     | S     | Ni     | Cr    | Mo     | Ca     | V     | Nb    |  |
| 1                                                   | 0.13  | 0.48   | 0.26 | 0.011 | 0.001 | 0.12   | 2.07  | 0.95   | 0.013  | <0.01 | <0.01 |  |
| 2                                                   | 0.14  | 0.46   | 0.24 | 0.011 | 0.001 | 0.11   | 2.14  | 0.95   | 0.010  | <0.01 | <0.01 |  |
| Pipe                                                | Ti    | N      | Cu   | Al    | As    | Sb     | Sn    | B      |        |       |       |  |
| 1                                                   | 0.001 | 0.0074 | 0.13 | 0.014 | 0.006 | 0.0013 | 0.007 | 0.0001 | 0.0002 |       |       |  |
| 2                                                   | 0.001 | 0.0083 | 0.13 | 0.014 | 0.006 | 0.0007 | 0.008 | 0.0001 | 0.0002 |       |       |  |

The as-rolled pipes were subsequently austenitized by heating to a temperature of about 920° C. for approximately 5400 sec by a walking beam furnace, descaled by high pressure water nozzles, and externally and internally water quenched using a tank with stirred water and an inner water nozzle. The austenitizing heating rate was approximately 0.16° C./s. The cooling rate employed during quenching was approximately 15° C./s. The quenched pipes were rapidly moved to another walking beam furnace for tempering treatment at a temperature of about 740° C. for a total time of about 9000 sec and a soaking time of about 4200 sec. The tempering heating rate was approximately 0.12° C./s. The cooling rate employed during tempering was approximately less than about 0.1° C./s. All the quenched and tempered (Q&T) pipes were hot straightened.

The main parameters characterizing the microstructure and non-metallic inclusions of the pipes of Example 1 are shown in Table 4.

TABLE 4

| Microstructural parameters of seamless pipes of example 1 |               |
|-----------------------------------------------------------|---------------|
| Parameter                                                 | Average value |
| Austenite grain size (μm)                                 | 47.8          |
| Packet size (μm)                                          | 5.8           |
| Martensite (volume %)                                     | 68            |
| Lower Bainite (volume %)                                  | 32            |
| Volume of non-metallic inclusions (%)                     | 0.028         |
| Inclusions with size > 15 μm (No./mm <sup>2</sup> )       | 0.22          |

The mechanical properties of the pipes of Example 1 are shown in Tables 5, 6, and 7. Table 5 presents the tensile, elongation, hardness, and toughness properties of the quenched and tempered pipes. Table 6 presents the yield strength, fracture appearance transition temperature, crack tip opening displacement, and ductility transition temperature after a simulated post-weld heat treatment. The post-weld heat treatment comprised heating and cooling at a rate of about 80° C./h to a temperature of about 690° C. with a soaking times of about 5 h. Table 7 presents the measured HIC and SSC resistance of the quenched and tempered pipes.

TABLE 5

| Mechanical properties of quenched and tempered pipes of example 1 |        |
|-------------------------------------------------------------------|--------|
| Mechanical Property                                               | Result |
| Average Yield Strength (MPa)                                      | 479    |
| Minimum Yield Strength (MPa)                                      | 466    |
| Maximum Yield Strength (MPa)                                      | 489    |
| Average Ultimate Tensile Strength, UTS (MPa)                      | 612    |
| Minimum Ultimate Tensile Strength, UTS (MPa)                      | 604    |
| Maximum Ultimate Tensile Strength, UTS (MPa)                      | 617    |
| Maximum YS/UTS ratio                                              | 0.81   |

TABLE 5-continued

| Mechanical properties of quenched and tempered pipes of example 1                |        |
|----------------------------------------------------------------------------------|--------|
| Mechanical Property                                                              | Result |
| Average Elongation (%)                                                           | 23.1   |
| Minimum Elongation (%)                                                           | 21.5   |
| Maximum Elongation (%)                                                           | 26.8   |
| Maximum Hardness (HV <sub>10</sub> )                                             | 212    |
| Average Impact Energy (J) at about -70° C. [transverse CVN specimens]            | 240    |
| Individual Minimum Impact Energy (J) at about -70° C. [transverse CVN specimens] | 150    |
| 80% FATT (° C.) [transverse CVN specimens]                                       | -80    |
| 50% FATT (° C.) [transverse CVN specimens]                                       | -100   |
| Average CTOD (mm) at about -60° C.                                               | 1.03   |
| Nil ductility transition temperature (° C.)                                      | ≤-80   |

TABLE 6

| Mechanical properties of quenched and tempered pipes of example 1 after simulated Post Weld Heat Treatment (PWHT1) |        |
|--------------------------------------------------------------------------------------------------------------------|--------|
| Parameter                                                                                                          | Result |
| Minimum Yield Strength (MPa) after PWHT1                                                                           | 462    |
| 50% FATT (° C.) [transverse CVN specimens] after PWHT1                                                             | -95    |
| Average CTOD (mm) at about -60° C. after PWHT1                                                                     | 2.4    |
| Nil ductility transition temperature (° C.) by DWT after PWHT1                                                     | ≤-95   |

TABLE 7

| HIC and SSC resistance of Q&T pipes of example 1 |                      |                 |
|--------------------------------------------------|----------------------|-----------------|
|                                                  | Result               | Number of tests |
| HIC:                                             |                      |                 |
| Crack Length Ratio, CLR %                        | 0                    | 12              |
| Crack Thickness Ratio, CTR %                     | 0                    | 12              |
| Crack Sensitivity Ratio, CSR %                   | 0                    | 12              |
| SSC (NACE TM0177 method A, stress: 90% SMYS):    |                      |                 |
| Failure time (h)                                 | >720<br>(all passed) | 12              |

It was found from the testing results above (Table 5, Table 6, and Table 7) that the quenched and tempered pipes are suitable to develop a 65 ksi grade, characterized by:

Yield strength (YS: about 450 MPa (65 ksi) minimum and about 600 MPa (87 ksi) maximum)  
 Ultimate Tensile Strength, UTS: about 535 MPa (78 ksi) minimum and about 760 MPa (110 ksi) maximum.  
 Hardness: about 248 HV<sub>10</sub> max.  
 Elongation, not less than about 20%.  
 YS/UTS ratio less than or equal to about 0.91.

Minimum Impact Energy of about 200 J/about 150 J (average/individual) at about  $-70^{\circ}\text{C}$ . on transverse Charpy V-notch specimens.

Excellent toughness in terms of 50% FATT (transition temperature for a fracture appearance with about 50% shear area) and about 80% FATT (transition temperature for a fracture appearance with about 80% shear area), measured on transverse Charpy V-notch specimens tested according with standard ISO 148-1.

Ductile-to-brittle transition temperature, measured by drop weight test (DWT) according with ASTM 208 standard, lower than about  $-70^{\circ}\text{C}$ .

Excellent longitudinal Crack Tip Opening Displacement (CTOD) at about  $-60^{\circ}\text{C}$ . ( $>0.8\text{ mm}$ ).

Yield strength (YS) of about 450 MPa minimum after simulated Post Weld Heat Treatment: heating and cooling rate of about  $80^{\circ}\text{C}/\text{h}$ , about  $650^{\circ}\text{C}$ . soaking temperature; soaking times: about 5 h. Good resistance to HIC (test according with NACE Standard TM0284-2003 Item No. 21215, using NACE solution A and test duration about 96 hours) and SSC (test in accordance with NACE TM0177, using test solution A and 1 bar  $\text{H}_2\text{S}$ , stressed at about 90% of specified minimum yield strength, SMYS).

## Example 2

### Microstructural and Mechanical Properties of Bends in Quenched and Tempered Thick-Wall Pipes

The quenched and tempered pipes of Example 1 were used to manufacture bends having a radius of approximately 5 times the outer diameter of the pipe (5 D).

The pipes were subjected to hot induction bending by heating to a temperature of approximately  $850^{\circ}\text{C}$ .  $+/-25^{\circ}\text{C}$ . and in-line water quenching. The bends were then reheated to a temperature of about  $920^{\circ}\text{C}$ . for approximately 15 min holding in a car furnace, moved to a water tank, and immersed in stirred water. The minimum temperature of the bends was higher than about  $860^{\circ}\text{C}$ . just before immersion in the water tank and the temperature of the water of the tank was maintained below approximately  $40^{\circ}\text{C}$ . The microstructure of the as-quenched bend at about the mid-wall of the pipe is illustrated in FIG. 7.

Following the quenching operation, the as-quenched bends were tempered in a furnace set at a temperature of about  $730^{\circ}\text{C}$ . using an approximately 40 min holding time.

TABLE 8

### Mechanical Properties of Quenched and Tempered Bends of Example 2

| Mechanical Property                                                                              | Result |
|--------------------------------------------------------------------------------------------------|--------|
| Average Yield Strength (MPa)                                                                     | 502    |
| Minimum Yield Strength (MPa)                                                                     | 485    |
| Maximum Yield Strength (MPa)                                                                     | 529    |
| Average Ultimate Tensile Strength, UTS (MPa)                                                     | 642    |
| Minimum Ultimate Tensile Strength, UTS (MPa)                                                     | 634    |
| Maximum Ultimate Tensile Strength, UTS (MPa)                                                     | 647    |
| Maximum YS/UTS ratio (—)                                                                         | 0.82   |
| Average Elongation (%)                                                                           | 22.0   |
| Minimum Elongation (%)                                                                           | 20.5   |
| Maximum Elongation (%)                                                                           | 25.0   |
| Maximum Hardness ( $\text{HV}_{10}$ )                                                            | 211    |
| Average Impact Energy (J) at about $-70^{\circ}\text{C}$ . [transverse CVN specimens]            | 270    |
| Individual Minimum Impact Energy (J) at about $-70^{\circ}\text{C}$ . [transverse CVN specimens] | 210    |
| 80% FATT ( $^{\circ}\text{C}$ ) [transverse CVN specimens]                                       | $<-90$ |

TABLE 8-continued

| Mechanical Properties of Quenched and Tempered Bends of Example 2 |           |  |
|-------------------------------------------------------------------|-----------|--|
| Mechanical Property                                               | Result    |  |
| 50% FATT ( $^{\circ}\text{C}$ ) [transverse CVN specimens]        | $<-110$   |  |
| Average CTOD (mm) at about $-45^{\circ}\text{C}$ .                | $>1.1$    |  |
| Nil ductility transition temperature ( $^{\circ}\text{C}$ )       | $\leq-80$ |  |

TABLE 11

| HIC and SSC Resistance of Quenched and Tempered Bends of Example 2 |                        |                 |
|--------------------------------------------------------------------|------------------------|-----------------|
|                                                                    | Result                 | Number of tests |
| HIC:                                                               |                        |                 |
| Crack Length Ratio, CLR %                                          | 0                      | 3               |
| Crack Thickness Ratio, CTR %                                       | 0                      | 3               |
| Crack Sensitivity Ratio, CSR %                                     | 0                      | 3               |
| SSC (NACE TM0177 method A, stress: 90% SMYS):                      |                        |                 |
| Failure time (h)                                                   | $>720$<br>(all passed) | 3               |

It was found from the testing results above (Table 8, Table 9) that the quenched and tempered pipes are suitable to develop a 70 ksi grade, characterized by:

Yield strength (YS): about 485 MPa (70 ksi) minimum and about 635 MPa (92 ksi) maximum

Ultimate Tensile Strength, UTS: about 570 MPa (83 ksi) minimum and about 760 MPa (110 ksi) maximum.

Maximum hardness: about 248  $\text{HV}_{10}$ .

Elongation, not less than about 8%.

YS/UTS ratio no higher than about 0.93.

Minimum Impact Energy of about 200 J/about 150 J (average/individual) at about  $-70^{\circ}\text{C}$ . on transverse Charpy V-notch specimens.

Excellent toughness in terms of 50% FATT (transition temperature for a fracture appearance with about 50% shear area) and 80% FATT (transition temperature for a fracture appearance with about 80% shear area), measured on transverse Charpy V-notch specimens.

Excellent longitudinal Crack Tip Opening Displacement (CTOD) at about  $-45^{\circ}\text{C}$ . ( $>1.1\text{ mm}$ ).

Good resistance to HIC (test according with NACE Standard TM0284-2003 Item No. 21215, using NACE solution A and test duration about 96 hours) and SSC (test in accordance with NACE TM0177, using test solution A and 1 bar  $\text{H}_2\text{S}$ , stressed at about 90% of specified minimum yield strength, SMYS).

## Example 3

### Comparative Example of Quenched and Tempered Pipe

In this comparative example, quenched and tempered pipes having an outer diameter of about 219.1 mm and wall thickness of about 44 mm, made of a typical line pipe steel with a low carbon equivalent of 0.4% (Table 10), were used to manufacture hot induction bends, off-line quench and temper, using embodiments of the process previously described.

TABLE 10

| Composition of Comparative Example 3 |       |        |      |       |       |        |      |        |       |      |        |  |
|--------------------------------------|-------|--------|------|-------|-------|--------|------|--------|-------|------|--------|--|
| Heat                                 | C     | Mn     | Si   | P     | S     | Ni     | Cr   | Mo     | Ca    | V    | Nb     |  |
| 976866                               | 0.09  | 1.17   | 0.26 | 0.012 | 0.002 | 0.41   | 0.17 | 0.15   | 0.012 | 0.07 | 0.030  |  |
| Heat                                 | Ti    | N      | Cu   | Al    | As    | Sb     | Sn   | B      |       |      | H      |  |
| 976866                               | 0.002 | 0.0055 | 0.14 | 0.024 | 0.006 | 0.0027 | 0.01 | 0.0002 |       |      | 0.0002 |  |

The produced seamless pipes, were austenitized at about 920° C. using a soaking time of about 600 sec, as discussed above, by a walking beam furnace. The pipes were further descaled by high pressure water nozzles and externally and internally water quenched using a tank with stirred water and an inner water nozzle. The quenched pipes were rapidly moved to another walking beam furnace for tempering treatment at about 660° C. to about 670° C. Each of the quenched and tempered pipes were hot straightened.

The Q&T pipes were further subjected to hot induction bending by heating to a temperature of about 850° C. +/- 25° C. and in-line water quenched. The bends were then reheated at about 920° C. for an approximately 30 min hold time in a car furnace, moved to a water tank and immersed in stirred water. The minimum temperature of the bends was greater than about 860° C. just before immersion in the water tank and the temperature of the water of the tank was maintained below about 40° C. The microstructure at about the mid-wall of the as-quenched bend is illustrated in FIG. 8.

A predominant microstructure within the as-quenched pipe was granular bainite (a mixture of bainitic dislocated-ferrite and islands of high C martensite and retained austenite, MA constituent), which is significantly different from that of the high Cr-high Mo steel in FIG. 7.

The as-quenched bends were further tempered in a furnace set at about 670° C. using an approximately 30 min holding time.

The main parameters which characterize the microstructure and non-metallic inclusions of the Q&T bends are shown in Table 11.

TABLE 11

| Microstructural Parameters of Comparative Example 3 |                         |
|-----------------------------------------------------|-------------------------|
| Parameter                                           | Average value           |
| Packet size (μm)                                    | >8                      |
| Granular Bainite (volume %)                         | 92<br>(included 14% MA) |
| Ferrite (volume %)                                  | 8                       |
| Volume of non-metallic inclusions (%)               | 0.033                   |
| Inclusions with size > 15 mm (No./mm <sup>2</sup> ) | 0.24                    |

TABLE 12

| Mechanical Properties of Quenched and Tempered Bends of Comparative Example 3 |        |
|-------------------------------------------------------------------------------|--------|
| Mechanical Property                                                           | Result |
| Average Yield Strength (MPa)                                                  | 501    |
| Minimum Yield Strength (MPa)                                                  | 465    |
| Maximum Yield Strength (MPa)                                                  | 542    |
| Average Ultimate Tensile Strength, UTS (MPa)                                  | 626    |
| Minimum Ultimate Tensile Strength, UTS (MPa)                                  | 598    |
| Maximum Ultimate Tensile Strength, UTS (MPa)                                  | 652    |
| Maximum YS/UTS ratio                                                          | 0.81   |

TABLE 12-continued

| Mechanical Properties of Quenched and Tempered Bends of Comparative Example 3    |        |
|----------------------------------------------------------------------------------|--------|
| Mechanical Property                                                              | Result |
| Average Elongation (%)                                                           | 21.5   |
| Minimum Elongation (%)                                                           | 20.5   |
| Maximum Elongation (%)                                                           | 24.0   |
| Maximum Hardness (HV <sub>10</sub> )                                             | 240    |
| Average Impact Energy (J) at about -70° C.<br>[transverse CVN specimens]         | 70     |
| Individual Minimum Impact Energy (J) at about -70° C. [transverse CVN specimens] | 30     |
| 80% FATT (° C.) [transverse CVN specimens]                                       | -50    |
| 50% FATT (° C.) [transverse CVN specimens]                                       | -60    |

TABLE 13

| HIC and SSC resistance of Q&T bends of Example 3 |                     |                  |
|--------------------------------------------------|---------------------|------------------|
|                                                  | Result              | Number of tests  |
| HIC:                                             |                     |                  |
| Crack Length Ratio, CLR %                        | 0                   | 3                |
| Crack Thickness Ratio, CTR %                     | 0                   | 3                |
| Crack Sensitivity Ratio, CSR %                   | 0                   | 3                |
| SSC (NACE TM0177 method A, stress:<br>90% SMYS): |                     |                  |
| Failure time (h)                                 | >720<br>562<br>>720 | 3 (1 not passed) |

From the forgoing, it may be observed that pipes having quenched and tempered bends, as they are manufactured with a steel that does not develop enough hardenability, exhibit a predominant granular bainite microstructure. Moreover, the packet size is larger than that of Example 2.

Moreover, while these quenched and tempered bends are able to achieve the minimum yield strength of 450 MPa, i.e. grade X65 (Table 12), they have a lower toughness with higher transition temperatures and a lower resistance to SSC, as compared to Example 2, due to their different microstructure.

Although the foregoing description has shown, described, and pointed out the fundamental novel features of the present teachings, it will be understood that various omissions, substitutions, and changes in the form of the detail of the apparatus as illustrated, as well as the uses thereof, may be made by those skilled in the art, without departing from the scope of the present teachings. Consequently, the scope of the present teachings should not be limited to the foregoing discussion, but should be defined by the appended claims.

What is claimed is:

1. A heavy wall seamless steel pipe, comprising:  
 a steel composition comprising:  
 about 0.05 wt. % to about 0.16 wt. % carbon;  
 about 0.20 wt. % to about 0.90 wt. % manganese;  
 about 0.10 wt. % to about 0.50 wt. % silicon;  
 about 1.20 wt. % to about 2.60 wt. % chromium;  
 about 0.05 wt. % to about 0.50 wt. % nickel;  
 about 0.80 wt. % to about 1.20 wt. % molybdenum;  
 about 0.005 wt. % to about 0.12 wt. % vanadium;  
 about 0.008 wt. % to about 0.04 wt. % aluminum;  
 about 0.0030 wt. % to about 0.0120 wt. % nitrogen; and  
 about 0.0010 wt. % to about 0.005 wt. % calcium;  
 wherein the remainder of the composition comprises  
 iron and impurities;  
 wherein the wall thickness of the steel pipe is greater than  
 or equal to 35 mm; and  
 wherein the steel pipe is processed to have a yield strength  
 greater than or equal to 450 MPa, wherein the micro-  
 structure of the steel pipe consists essentially of marten-  
 site and lower bainite, wherein martensite is in a volume  
 percentage greater than or equal to 50% and lower bain-  
 ite is in a volume percentage less than or equal to 50%,  
 and wherein the steel pipe does not exhibit failure due at  
 least in part to stress corrosion cracking after 720 hours  
 when subjected to a stress of 90% of the yield stress and  
 tested according to NACE TM0177.
2. The steel pipe of claim 1, wherein the steel composition  
 further comprises:  
 about 0 to 0.80 wt. % tungsten;  
 about 0 to 0.030 wt. % niobium;  
 about 0 to 0.020 wt. % titanium;  
 about 0 to about 0.30 wt. % copper;  
 about 0 to about 0.010 wt. % sulfur;  
 about 0 to about 0.020 wt. % phosphorus;  
 about 0 to about 0.0020 wt. % boron;  
 about 0 to about 0.020 wt. % arsenic;  
 about 0 to about 0.0050 wt. % antimony;  
 about 0 to about 0.020 wt. % tin;  
 about 0 to about 0.030 wt. % zirconium;  
 about 0 to about 0.030 wt. % tantalum;  
 about 0 to about 0.0050 wt. % bismuth;  
 about 0 to about 0.0030 wt. % oxygen; and  
 about 0 to about 0.00030 wt. % hydrogen;  
 wherein the remainder of the composition comprises iron  
 and impurities.

3. The steel pipe of claim 2, wherein the steel composition  
 comprises:  
 about 0.07 wt. % to about 0.14 wt. % carbon;  
 about 0.30 wt. % to about 0.60 wt. % manganese;  
 about 0.10 wt. % to about 0.40 wt. % silicon;  
 about 1.80 wt. % to about 2.50 wt. % chromium;  
 about 0.05 wt. % to about 0.20 wt. % nickel;  
 about 0.90 wt. % to about 1.10 wt. % molybdenum;  
 about 0 to about 0.60 wt. % tungsten;  
 about 0 to about 0.015 wt. % niobium;  
 about 0 to about 0.010 wt. % titanium;  
 about 0 to about 0.20 wt. % copper;  
 about 0 to about 0.005 wt. % sulfur;  
 about 0 to about 0.012 wt. % phosphorus;  
 about 0.050 wt. % to about 0.10 wt. % vanadium;  
 about 0.010 wt. % to about 0.030 wt. % aluminum;  
 about 0.0030 wt. % to about 0.0100 wt. % nitrogen;  
 about 0.0010 wt. % to about 0.003 wt. % calcium;  
 about 0.0005 wt. % to about 0.0012 wt. % boron;  
 about 0 to about 0.015 wt. % arsenic;  
 about 0 to about 0.0050 wt. % antimony;

- about 0 to 0.015 wt. % tin;  
 about 0 to about 0.015 wt. % zirconium;  
 about 0 to about 0.015 wt. % tantalum;  
 about 0 to about 0.0050 wt. % bismuth;  
 about 0 to 0.0020 wt. % oxygen; and  
 about 0 to 0.00025 wt. % hydrogen;  
 wherein remainder of the composition comprises iron and  
 impurities.
4. The steel pipe of claim 2, wherein the steel composition  
 comprises:  
 about 0.08 wt. % to about 0.12 wt. % carbon;  
 about 0.30 wt. % to about 0.50 wt. % manganese;  
 about 0.10 wt. % to about 0.25 wt. % silicon;  
 about 2.10 wt. % to about 2.40 wt. % chromium;  
 about 0.05 wt. % to about 0.20 wt. % nickel;  
 about 0.95 wt. % to about 1.10 wt. % molybdenum;  
 about 0 to about 0.30 wt. % tungsten;  
 about 0 to about 0.010 wt. % niobium;  
 about 0 to about 0.010 wt. % titanium;  
 about 0 to about 0.15 wt. % copper;  
 about 0 to about 0.003 wt. % sulfur;  
 about 0 to about 0.010 wt. % phosphorus;  
 about 0.050 wt. % to about 0.07 wt. % vanadium;  
 about 0.015 wt. % to about 0.025 wt. % aluminum;  
 about 0.0030 wt. % to about 0.008 wt. % nitrogen;  
 about 0.0015 wt. % to about 0.003 wt. % calcium;  
 about 0.0008 wt. % to about 0.0014 wt. % boron;  
 about 0 to about 0.015 wt. % arsenic;  
 about 0 to about 0.0050 wt. % antimony;  
 about 0 to about 0.015 wt. % tin;  
 about 0 to about 0.010 wt. % zirconium;  
 about 0 to about 0.010 wt. % tantalum;  
 about 0 to about 0.0050 wt. % bismuth;  
 about 0 to about 0.0015 wt. % oxygen; and  
 about 0 to about 0.00020 wt. % hydrogen;  
 wherein the remainder of the composition comprises iron  
 and impurities.
5. The steel pipe of claim 1, wherein the pipe is processed  
 to have a yield strength greater than or equal to 485 MPa.
6. The steel pipe of claim 1, wherein the microstructure of  
 the steel pipe does not include one or more of ferrite, upper  
 bainite, and granular bainite.
7. The steel pipe of claim 1, wherein the volume percentage  
 of martensite is greater than or equal to 90% and the volume  
 percentage of lower bainite is less than or equal to 10%.
8. The steel pipe of claim 1, wherein the steel pipe has a  
 prior austenite grain size between about 15  $\mu\text{m}$  and about 100  
 $\mu\text{m}$ .
9. The steel pipe of claim 1, wherein the steel pipe has a  
 packet size less than or equal to 6  $\mu\text{m}$ .
10. The steel pipe of claim 1, further comprising one or  
 more particulates having a composition of the form MX or  
 $\text{M}_2\text{X}$ , wherein an average diameter of the one or more particulates  
 is less than or equal to 40 nm and wherein M is  
 selected from V, Mo, Nb, and Cr and X is selected from C and  
 N.
11. The steel pipe of claim 1, wherein the steel pipe has a  
 ductile to brittle transition temperature less than  $-70^\circ\text{C}$ .
12. The steel pipe of claim 1, wherein the steel pipe has a  
 Charpy V-notch energy greater or equal to 150 J/cm<sup>2</sup>.
13. A method of making a heavy wall steel pipe, comprising:  
 providing a steel having a carbon steel composition com-  
 prising:  
 about 0.05 wt. % to about 0.16 wt. % carbon;  
 about 0.20 wt. % to about 0.90 wt. % manganese;  
 about 0.10 wt. % to about 0.50 wt. % silicon;

27

about 1.2 wt. % to about 2.6 wt. % chromium;  
 about 0.05 wt. % to about 0.50 wt. % nickel;  
 about 0.80 wt. % to about 1.2 wt. % molybdenum;  
 about 0.005 wt. % to about 0.12 wt. % vanadium;  
 about 0.008 wt. % to about 0.04 wt. % aluminum;  
 about 0.0030 wt. % to about 0.0120 wt. % nitrogen; and  
 about 0.0010 wt. % to about 0.005 wt. % calcium;  
 wherein the remainder of the composition comprises  
 iron and impurities;  
 forming the steel into a tube having a wall thickness greater  
 than or equal to 35 mm;  
 heating the formed steel tube in a first heating operation to  
 a temperature within the range between about 900° C. to  
 about 1060° C.;  
 quenching the formed steel tube at a rate greater than or  
 equal to 7° C./sec, wherein the microstructure of the  
 quenched steel consists essentially of martensite and  
 lower bainite, wherein martensite is in a volume percent-  
 age greater than or equal to 50% and lower bainite is in  
 a volume percentage less than or equal to 50% and  
 wherein the microstructure has an average prior austen-  
 ite grain size greater than 15  $\mu\text{m}$ ; and  
 tempering the quenched steel tube at a temperature within  
 the range between about 680° C. to about 760° C.;  
 wherein, after tempering, the steel tube has a yield strength  
 greater than 450 MPa and a Charpy V-notch energy  
 greater than or equal to 150 J/cm<sup>2</sup>.

14. The method of claim 13, wherein the steel composition  
 further comprises:

about 0 to about 0.80 wt. % tungsten;  
 about 0 to about 0.030 wt. % niobium;  
 about 0 to about 0.020 wt. % titanium;  
 about 0 to about 0.0020 wt. % boron;  
 about 0 to about 0.020 wt. % arsenic;  
 about 0 to about 0.0050 wt. % antimony;  
 about 0 to about 0.020 wt. % tin;  
 about 0 to about 0.030 wt. % zirconium;  
 about 0 to about 0.030 wt. % tantalum;  
 about 0 to about 0.0050 wt. % bismuth;  
 about 0 to about 0.0030 wt. % oxygen; and  
 about 0 to about 0.00030 wt. % hydrogen;  
 wherein the remainder of the composition comprises iron  
 and impurities.

15. The method of claim 14, wherein the steel composition  
 comprises:

about 0.07 wt. % to about 0.14 wt. % carbon;  
 about 0.30 wt. % to about 0.60 wt. % manganese;  
 about 0.10 wt. % to about 0.40 wt. % silicon;  
 about 1.80 wt. % to about 2.50 wt. % chromium;  
 about 0.05 wt. % to about 0.20 wt. % nickel;  
 about 0.90 wt. % to about 1.10 wt. % molybdenum;  
 about 0 to about 0.60 wt. % tungsten;  
 about 0 to about 0.015 wt. % niobium;  
 about 0 to about 0.010 wt. % titanium;  
 about 0 to about 0.20 wt. % copper;  
 about 0 to about 0.005 wt. % sulfur;  
 about 0 to about 0.012 wt. % phosphorus;  
 about 0.050 wt. % to about 0.10 wt. % vanadium;  
 about 0.010 wt. % to about 0.030 wt. % aluminum;  
 about 0.0030 wt. % to about 0.0100 wt. % nitrogen; and  
 about 0.0010 wt. % to 0.003 wt. % calcium;  
 about 0.0005 wt. % to 0.0012 wt. % boron;  
 about 0 to about 0.015 wt. % arsenic;  
 about 0 to about 0.0050 wt. % antimony;  
 about 0 to about 0.015 wt. % tin;  
 about 0 to about 0.015 wt. % zirconium;  
 about 0 to about 0.015 wt. % tantalum;

28

about 0 to about 0.0050 wt. % bismuth;  
 about 0 to about 0.0020 wt. % oxygen; and  
 about 0 to about 0.00025 wt. % hydrogen;  
 wherein the remainder of the composition comprises iron  
 and impurities.

16. The method of claim 15, wherein the steel composition  
 comprises:

about 0.08 wt. % to about 0.12 wt. % carbon;  
 about 0.30 wt. % to about 0.50 wt. % manganese;  
 about 0.10 wt. % to about 0.25 wt. % silicon;  
 about 2.10 wt. % to about 2.40 wt. % chromium;  
 about 0.05 wt. % to about 0.20 wt. % nickel;  
 about 0.95 wt. % to about 1.10 wt. % molybdenum;  
 about 0 to about 0.30 wt. % tungsten;  
 about 0 to about 0.010 wt. % niobium;  
 about 0 to about 0.010 wt. % titanium;  
 about 0.050 wt. % to about 0.07 wt. % vanadium;  
 about 0.015 wt. % to about 0.025 wt. % aluminum;  
 about 0 to about 0.15 wt. % copper;  
 about 0 to about 0.003 wt. % sulfur;  
 about 0 to about 0.010 wt. % phosphorus;  
 about 0.0030 wt. % to about 0.008 wt. % nitrogen; and  
 about 0.0015 wt. % to about 0.003 wt. % calcium;  
 about 0.0008 wt. % to about 0.0014 wt. % boron;  
 about 0 to about 0.015 wt. % arsenic;  
 about 0 to 0.0050 wt. % antimony;  
 about 0 to 0.015 wt. % tin;  
 about 0 to about 0.010 wt. % zirconium; and  
 about 0 to about 0.010 wt. % tantalum;  
 about 0 to about 0.0050 wt. % bismuth;  
 about 0 to about 0.0015 wt. % oxygen; and  
 about 0 to about 0.00020 wt. % hydrogen; and  
 wherein the remainder of the composition comprises iron  
 and impurities.

17. The method of claim 13, wherein, after quenching, the  
 steel tube has a yield strength greater than 485 MPa.

18. The method of claim 13, wherein the microstructure of  
 the steel tube does not include one or more of ferrite, upper  
 bainite, and granular bainite.

19. The method of claim 13, wherein the volume percent-  
 age of martensite is greater than or equal to 90% and the  
 volume percentage of lower bainite is less than or equal to  
 10%.

20. The method of claim 13, wherein, after quenching, a  
 packet size of the steel tube is less than or equal to 6  $\mu\text{m}$ .

21. The method of claim 13, wherein, after tempering, the  
 steel tube further comprises one or more particulates having  
 the composition MX or M<sub>2</sub>X, wherein the one or more partic-  
 culates have an average diameter less than or equal to 40  $\mu\text{m}$   
 and wherein M is selected from V, Mo, Nb, and Cr and X is  
 selected from C and N.

22. The method of claim 13, wherein, after tempering, the  
 steel tube has a ductile to brittle transition temperature less  
 than -70° C.

23. The steel pipe of claim 1, wherein the steel comprises  
 about 1.80 wt. % to about 2.60 wt. % chromium.

24. The steel pipe of claim 1, wherein the steel pipe has a  
 maximum hardness of about 248 HV<sub>10</sub>.

25. The method of claim 13, wherein, after tempering, the  
 steel tube has a maximum hardness of about 248 HV<sub>10</sub>.

26. A method of making a heavy wall steel pipe, comprising:  
 providing a steel having a carbon steel composition com-  
 prising:  
 0.05 wt. % to about 0.16 wt. % carbon+/-less than 10%;  
 0.20 wt. % to about 0.90 wt. % manganese+/-less than  
 10%;

**29**

0.10 wt. % to about 0.50 wt. % silicon+/-less than 10%;  
 1.80 wt. % to about 2.60 wt. % chromium+/-less than 10%;  
 0.05 wt. % to about 0.50 wt. % nickel+/-less than 10%;  
 0.80 wt. % to about 1.20 wt. % molybdenum+/-less than 10%;  
 0.005 wt. % to about 0.12 wt. % vanadium+/-less than 10%;  
 0.008 wt. % to about 0.04 wt. % aluminum+/-less than 10%;  
 0.0030 wt. % to about 0.0120 wt. % nitrogen+/-less than 10%; and  
 0.0010 wt. % to about 0.005 wt. % calcium+/-less than 10%;  
 wherein the remainder of the composition comprises 15  
 iron and impurities;  
 forming the steel into a tube having a wall thickness greater than or equal to 35 mm;  
 heating the formed steel tube in a first heating operation to a temperature within the range between about 900° C. to about 1060° C.;

**30**

quenching the formed steel tube at a rate greater than or equal to 7° C./sec, wherein the microstructure of the quenched steel is, in a volume percentage greater than or equal to 50% martensite and less than or equal to 50% lower bainite and wherein the microstructure has an average prior austenite grain size greater than 15  $\mu\text{m}$ ; and

tempering the quenched steel tube at a temperature within the range between about 680° C. to about 760° C.; wherein, after tempering, the steel tube has a yield strength greater than 450 MPa and a Charpy V-notch energy greater than or equal to 150 J/cm<sup>2</sup>, and wherein the steel pipe does not exhibit failure due at least in part to stress corrosion cracking after 720 hours when subjected to a stress of 90% of the yield stress and tested according to NACE TM0177.

**27.** The method of claim **26**, wherein, after tempering, the steel tube has a maximum hardness of about 248 HV<sub>10</sub>.

\* \* \* \* \*

UNITED STATES PATENT AND TRADEMARK OFFICE  
**CERTIFICATE OF CORRECTION**

PATENT NO. : 8,821,653 B2  
APPLICATION NO. : 13/367312  
DATED : September 2, 2014  
INVENTOR(S) : Ettore Anelli

Page 1 of 2

It is certified that error appears in the above-identified patent and that said Letters Patent is hereby corrected as shown below:

Title page (item 57, Abstract) at line 14, Change “485” to --485 MPa--.

In column 1 (title page 3, item 56) at line 48, Under Other Publications, change “Pergamom” to --Pergamon--.

In column 2 (title page 3, item 56) at line 52, Under Other Publications, change “Tublar” to --Tubular--.

In column 2 (title page 3, item 56) at line 58, Under Other Publications, change “Kokan” to --Konkan--.

In column 1 (title page 4, item 56) at line 14, Under Other Publications, change “Baintitic” to --Bainitic--.

In column 1 (title page 4, item 56) at line 20, Under Other Publications, change “microstruture” to --microstructure--.

In column 1 (title page 4, item 56) at line 23, Under Other Publications, change “Moessbauer” to --“Mossbauer--.

In column 1 (title page 4, item 56) at line 35, Under Other Publications, change “Spinger-Verlag,” to --Springer-Verlag, --.

In column 2 (title page 4, item 56) at line 8, Under Other Publications, change “Moessbauer” to --Mossbauer--.

In column 2 (title page 4, item 56) at line 36, Under Other Publications, change “Tempuratures”,” to --Temperatures”,--.

In the Specification

In column 4 at line 2, Change “vanadium” to --vanadium;--.

In column 4 at line 5 (approx.), Change “calcium:” to --calcium;--.

Signed and Sealed this  
Twenty-fourth Day of March, 2015



Michelle K. Lee  
Director of the United States Patent and Trademark Office

**CERTIFICATE OF CORRECTION (continued)**  
**U.S. Pat. No. 8,821,653 B2**

Page 2 of 2

In column 6 at line 7, Change “0.80%” to --0.80%;--.  
In column 6 at line 64, Change “X=C” to --X=C--.  
In column 7 at line 38, Change “(MC).” to --(HIC).--.  
In column 13 at line 20, Change “1.340° C.,” to --1340° C.,--.  
In column 13 at line 24, Change “Manessmann” to --Mannesmann--.  
In column 13 at line 28, Change “Manessmann” to --Mannesmann--.  
In column 16 at line 48, Change “may, be” to --may be--.  
In column 18 at line 52 (approx.), Change “in, a” to --in a--.  
In column 22 at line 12 (approx.), Change “TABLE 11” to --TABLE 9--.  
In column 22 at line 30 (approx.), Change “maximum” to --maximum.--.

In the Claims

In column 28 at line 65, In Claim 26, change “carbon+/-less” to --carbon +/- less--.  
In column 28 at line 66, In Claim 26, change “manganese+/-less” to --manganese +/- less--.  
In column 29 at line 1, In Claim 26, change “silicon+/-less” to --silicon +/- less--.  
In column 29 at line 2, In Claim 26, change “chromium+/-less” to --chromium +/- less--.  
In column 29 at line 4, In Claim 26, change “nickel+/-less” to --nickel +/- less--.  
In column 29 at line 5 (approx.), In Claim 26, change “molybdenum+/-less” to  
--molybdenum +/- less--.  
In column 29 at line 7 (approx.), In Claim 26, change “vanadium+/-less” to  
--vanadium +/- less--.  
In column 29 at line 9 (approx.), In Claim 26, change “aluminum+/-less” to  
--aluminum +/- less--.  
In column 29 at line 11 (approx.), In Claim 26, change “nitrogen+/-less” to  
--nitrogen +/- less--.  
In column 29 at line 13 (approx.), In Claim 26, change “calcium+/-less” to  
--calcium +/- less--.